# EUROPEAN PATENT APPLICATION

(11) **EP 4 682 285 A1**
(43) Date of publication of application: **21.01.2026**
(21) Application number: 24771022.1
(22) Date of filing: 15.03.2024
(51) Int. Cl.: C22C 38/00, C21D 8/02, C21D 9/00, C21D 9/46, C21D 9/50, C22C 38/08, C22C 38/58

(54) **STEEL**

(30) Priority: 16.03.2023 JP 2023042399; 16.03.2023 JP 2023042402
(71) Applicant: NIPPON STEEL CORPORATION, Chiyoda-ku Tokyo 100-8071 (JP)
(72) Inventor: UCHIYAMA, Tetsuya, Tokyo 100-8071 (JP); NAKANISHI, Daiki, Tokyo 100-8071 (JP); USUKI, Hirokazu, Tokyo 100-8071 (JP); SHIRAHATA, Hiroyuki, Tokyo 100-8071 (JP); YOSHIMURA, Nobuyuki, Tokyo 100-8071 (JP)
(74) Representative: Vossius & Partner Patentanwälte Rechtsanwälte mbB
(86) International application number: PCT/JP2024/010386
(87) International publication number: WO 2024/190920

(57) **Abstract**

A steel product having a specific chemical composition, in which α expressed by a following formula is 5.0 or more and 16.0 or less; having a tensile strength of 615 MPa or more and 930 MPa or less; and having a microstructure in a region that is 1/4 of a thickness from a surface that contains lower bainite and martensite, with a total of area ratios of the lower bainite and the martensite being 15.0% or more, a total of area ratios of upper bainite, the lower bainite, and the martensite being 90.0% or more, and an area ratio of residual austenite being less than 1.7%. α = 0.50 × √[C] × (1+0.64[Si]) × (1+4.10[Mn]) × (1+0.27[Cu]) × (1+0.52[Ni]) × (1+2.33[Cr]) × (1+3.14[Mo])

## Description

### Technical Field

The present disclosure relates to a steel product.

### Background Art

Steel products can be used in welded structures such as buildings, bridges, ships, pipelines, offshore structures, pressure vessels and tanks. Steel products having excellent strength and adaptability to low-temperature toughness are effective in low-temperature applications.

Cryogenic steel is used in cryogenic pressure vessels such as storage tanks for liquefied gases. Al-killed steel, nickel steel, high-Mn steel, austenitic stainless steel and the like exist in a cryogenic steel, in accordance with the usage temperature. For example, nickel steel such as 3.5% Ni steel is used as a material for tanks that store liquefied ethane or liquefied ethylene whose usage temperatures are around -100°C.

As with this 3.5% Ni steel, steel products that require ensured low-temperature toughness-exemplified by those used in cryogenic pressure vessels-are often made to contain Ni.

For example, Patent Document 1 proposes a nickel-containing steel product for low temperatures that has excellent toughness and has a specific chemical composition containing 2.7% or more and 5.0% or less Ni, wherein the prior austenite grain diameter at the time of quenching heating is 20 µm or less, and the effective crystal grain diameter after a heat treatment is 12 µm or less, and the tensile strength is 450 MPa or more and 690 MPa or less.

Further, various steel products of prescribed chemical compositions and microstructures (metal structures) have been proposed for the purposes of low-temperature toughness and high strength (see, for example, Patent Documents 2 through 6).
Patent Document 1: Japanese Patent Application Laid-Open (JP-A) No. 2019-81930
Patent Document 2: JP-A No. H06-192729
Patent Document 3: JP-A No. H07-331328
Patent Document 4: International Publication No. 2007/034576
Patent Document 5: International Publication No. 2020/184162
Patent Document 6: International Publication No. 2014/017057

### SUMMARY OF INVENTION

### Technical Problem

Having both high strength and the ensuring of low-temperature toughness is desirable for cryogenic steels that are used in cryogenic pressure vessels. Further, a cryogenic pressure vessel is manufactured by welding a steel product, and, in order to eliminate residual stress that arises due to the welding, there are cases in which a post weld heat treatment (called PWHT upon occasion) is carried out. Recently, the demand for low-temperature toughness of steel products after PWHT has increased even more.

A topic of the present disclosure is the provision of a steel product that is suited to low-temperature applications and that has good low-temperature toughness regardless of whether before or after a post weld heat treatment.

### Solution to Problem

The gist of the present disclosure is as follows.
<1> A steel product having a chemical composition including, in mass%,
   C: 0.03% or more and 0.20% or less,
   Si: 0.01% or more and 0.50% or less,
   Mn: 0.10% or more and 2.00% or less,
   P: 0.025% or less,
   S: 0.0250% or less,
   Ni: 4.51% or more and 6.10% or less,
   Al: 0.001% or more and 0.100% or less,
   O: 0.0100% or less,
   N: 0.0100% or less,
   Cu: 0 - 1.50%,
   Cr: 0 - 3.00%,
   Mo: 0 - 2.00%,
   B: 0 - 0.0050%,
   Nb: 0 - 0.050%,
   Ti: 0 - 0.050%,
   V: 0 - 0.10%,
   Mg: 0 - 0.0200%,
   Ca: 0 - 0.0200%,
   REM: 0 - 0.0200%,
   balance: Fe and impurities,
   and in which α expressed by following formula (1) is 5.0 or more and 16.0 or less,
   wherein:
      a tensile strength is 615 MPa or more and 930 MPa or less, and
      a microstructure of a region that is 1/4 of a thickness in a thickness direction from a surface of the steel product contains lower bainite and martensite, and a total of area ratios of the lower bainite and the martensite is 15.0% or more, and a total of area ratios of upper bainite and the lower bainite and the martensite is 90.0% or more, and an area ratio of residual austenite is less than 1.7%. α = 0.50 × √[C] × (1+0.64[Si]) × (1+4.10[Mn]) × (1+0.27[Cu]) × (1+0.52[Ni]) × (1+2.33[Cr]) × (1+3.14[Mo])
      wherein [element symbol] in formula (1) represents content (mass%) of a respectively corresponding element contained in the steel product, and, in a case in which an element is not contained, zero is substituted in therefor.
<2> The steel product of <1>, wherein, in the microstructure of the region that is 1/4 of the thickness in the thickness direction from the surface of the steel product, an average crystal grain diameter is 20.0 µm or less.
<3> The steel product of <1> or <2>, wherein a Charpy impact absorption energy at -110°C is 150 J or more.
<4> The steel product of any one of <1> through <3>, wherein, in a case in which a heat treatment, in which a rate of temperature increase and a rate of temperature decrease in a temperature region of 425°C or more are 55°C/h and temperature is held for 2 hours at 600°C, is carried out on the steel product, a Charpy impact absorption energy at -110°C of portions where the heat treatment has been carried out is 150 J or more.
<5> The steel product of any one of <1> through <4>, wherein an aspect ratio of prior austenite crystal grains of the region that is 1/4 of the thickness in the thickness direction from the surface of the steel product is 1.5 or more.
<6> The steel product of any one of <1> through <4>, wherein an aspect ratio of prior austenite crystal grains of the region that is 1/4 of the thickness in the thickness direction from the surface of the steel product is less than 1.5.

### Advantageous Effects of Invention

In accordance with the present disclosure, a steel product that is suited to low-temperature applications and that has good low-temperature toughness regardless of whether before or after a post weld heat treatment can be provided.

### BRIEF DESCRIPTION OF DRAWINGS

Fig. 1 is a diagram illustrating an example of results of discriminating the microstructure.

### DESCRIPTION OF EMBODIMENTS

The present disclosure is described in detail hereinafter.

The "post weld heat treatment" in the present disclosure means a post weld heat treatment based on the contents prescribed in JIS Z 3700:2009 "Method of post weld heat treatment Method", unless otherwise specified.

The "steel product" and the "base metal" in the present disclosure mean the steel product portion that does not include a surface treated layer such as a plating layer or a coated film. However, a surface treated layer such as a plating layer or a coated film may be formed on the surface of the steel product relating to the present disclosure. Further, the "base metal" in a welded joint means the steel product portion that is not affected by welding, in contrast to the welded portion (the welded metal or the heat affected zone).

In the present disclosure, numerical ranges expressed by using "-" mean ranges in which the numerical values listed before and after the "-" are included as the lower limit value and upper limit value, respectively. However, numerical value ranges in which "exceeds" or "less than" is appended to the numerical value listed before or after the "-" mean a range in which these numerical values are not included as the lower limit value or the upper limit value.

With respect to the contents of the elements in a chemical composition, "%" means "mass%".

The term "step" is not only an independent step and includes steps that, even in a case in which that step cannot be clearly distinguished from another step, achieve the intended object of that step.

A steel product relating to an embodiment of the present disclosure is described hereinafter. The new knowledge, which was obtained as the result of studies by the inventors of the present disclosure and which was arrived at in completing the steel product relating to the present disclosure, is described in detail first.

The inventors of the present disclosure carried out studies in order to improve the strength of steel products. The tensile strength of a steel product is ensured by the configuration of the microstructure. The inventors of the present disclosure took samples from a 1/4t portion (t: thickness of the steel product) of a steel product after hot rolling and accelerated cooling, and carried out tensile test thereon, and observed the microstructures. As a result, it was learned that, at the microstructure of the 1/4t portion of a steel product having a tensile strength of 615 MPa or more and 930 MPa or less, the area ratio of ferrite is less than 10.0%, and the total of the area ratios of upper bainite, lower bainite and martensite is 90.0% or more. Note that the total of the area ratios of upper bainite, lower bainite and martensite was measured by using electron back scatter diffraction (hereinafter called "EBSD").

Further, the inventors of the present disclosure carried out studies in order to improve the toughness of steel products. The toughness of a steel product is ensured by the configuration of the microstructure. The inventors of the present disclosure took samples from the 1/4t portion of a steel product after hot rolling and accelerated cooling, and carried out Charpy impact test, and observed the microstructures. As a result, it was found that, in a steel product exhibiting a Charpy impact absorption energy of 150 J or more at -110°C, the total of the area ratios of lower bainite and martensite is 15.0% or more and the area ratio of the residual austenite is less than 1.7%. Note that the total of the area ratios of lower bainite and martensite was measured by using EBSD. Note that the area ratio of the residual austenite was measured by X-ray diffraction. The volume ratio of the residual austenite measured by the X-ray diffraction may be considered to be the area ratio.

Moreover, the inventors of the present disclosure carried out studies in order to ensure the toughness of steel products. The toughness of a steel product is ensured by making the region, at which the difference in crystal orientation is 15° or more and which is surrounded by a high angle grain boundary, small. The inventors of the present disclosure took samples from the 1/4t portion of a steel product manufactured by controlling the cooling rate and the cooling stoppage temperature after hot rolling, and measured the circle equivalent diameter of the region surrounded by a high angle grain boundary by EBSD. The circle equivalent diameter of the region surrounded by a high angle grain boundary is called the crystal grain diameter hereinafter. The sample was subjected to mechanical polishing and electrolytic polishing, and analysis was carried out on a 4 mm² region by an EBSD device equipped with an FE-SEM (field emission scanning electron microscope). The value calculated by an area weighted average that was weighted by the area per crystal grain among the crystal grain diameters measured in the 4 mm² region, was used as the average crystal grain diameter (also called "effective crystal grain diameter" upon occasion). It was learned that, if the average crystal grain diameter of a 1/4t portion of a steel product is 20.0 µm or less, there is the tendency for the toughness of the steel product to improve more regardless of whether before or after a post weld heat treatment.

Further, the inventors of the present disclosure have found that similar results can be obtained not only with steel products after hot rolling and accelerated cooling, but also with steel products after reheat quenching.

### <Chemical Composition>

Alloy elements that constitute the chemical composition of the steel product relating to the present disclosure are described next. Note that, in the following description of the alloy elements, the "%" of the content means "mass%".

### (C: 0.03% or more and 0.20% or less)

C is an element that improves the strength of the steel product. From the standpoint of ensuring the strength of the steel product that is used in a structure, in the present disclosure, the C content is 0.03% or more. The C content is preferably 0.05% or more, or 0.07% or more. On the other hand, C is an element that reduces toughness, and, from the standpoint of ensuring the toughness of the heat affected zone (hereinafter called "HAZ" upon occasion), in the present disclosure, the C content is 0.20% or less. The C content is preferably 0.16% or less, 0.14% or less, or 0.12% or less.

### (Si: 0.01% or more and 0.50% or less)

Si is an element that is used as a deoxidizing agent, and further, that dissolves into the steel and increases the strength. From the standpoint of controlling the O concentration contained in molten steel, in the present disclosure, the Si content is 0.01% or more. The Si content is preferably 0.03% or more, 0.05% or more, 0.10% or more, or 0.12% or more. On the other hand, if the Si content is excessive, there are cases in which a hard phase forms in the HAZ, and the toughness decreases. Accordingly, from the standpoint of ensuring the toughness of the HAZ, in the present disclosure, the Si content is 0.50% or less. The Si content is preferably 0.30% or less, or 0.20% or less.

### (Mn: 0.10% or more and 2.00% or less)

Mn is an element that is used as a deoxidizing agent, and further, that improves the hardenability of the steel and contributes to increasing the strength. From the standpoint of controlling the O concentration contained in molten steel, in the present disclosure, the Mn content is 0.10% or more. Moreover, due to Mn in an amount of 0.10% or more, by forming MnS, the solid-solution S is reduced, and hot cracking is prevented. From the standpoint of ensuring the strength of the steel product and the toughness of the HAZ, the Mn content is preferably 0.30% or more, or 0.50% or more. On the other hand, if the Mn content is excessive, there are cases in which the toughness after PWHT decreases due to the Mn segregating at the grain boundary at the time of PWHT. Accordingly, from the standpoint of ensuring the toughness of the steel product after PWHT, in the present disclosure, the Mn content is 2.00% or less. The Mn content is preferably 1.80% or less, or 1.50% or less.

### (P: 0.025% or less)

P is an impurity element. Although the lower limit of the P content is not limited, from the standpoint of the manufacturing cost, in the present disclosure, the P content may be 0.001% or more. On the other hand, if the P content is excessive, there are cases in which the toughness after PWHT decreases due to the P segregating at the grain boundary at the time of PWHT. Accordingly, in the present disclosure, the P content is 0.025% or less. The P content is preferably 0.016% or less, 0.012% or less, or 0.008% or less.

### (S: 0.0250% or less)

S is an impurity element. Although the lower limit of the S content is not limited, from the standpoint of the manufacturing cost, in the present disclosure, the S content may be 0.0001% or more. On the other hand, if the S content is excessive, there are cases in which elongated MnS is generated at the centerline segregation area, and the toughness and ductility of the steel product and the HAZ deteriorate. From the standpoint of ensuring the toughness and ductility of the steel product and the HAZ, the S content is 0.0250% or less. The S content is preferably 0.0100% or less or 0.0050% or less.

### (Ni: 4.51% or more and 6.10% or less)

Ni is an element that is effective in improving the hardenability and toughness of the steel. Therefore, in the present embodiment, the Ni content is 4.51% or more. The Ni content is preferably 5.00% or more, or 5.25% or more. However, Ni is an expensive element, and, from the standpoint of cost reduction, in the present disclosure, the Ni content is 6.10% or less. The Ni content is preferably 6.00% or less, or 5.75% or less.

### (Al: 0.001% or more and 0.100% or less)

Al is an element that is effective in deoxidation, and is an element that, by forming a nitride, refines the crystal grain diameter at the time of quenching. Therefore, in the present disclosure, the Al content is 0.001% or more. However, if Al is excessively contained, there is the concern that the Al will generate a coarse nitride, and the toughness of the steel product and the HAZ will decrease. Accordingly, the Al content is 0.100% or less. The Al content is preferably 0.080%, or 0.050% or less.

### (O: 0.0100% or less)

O is an impurity element. Although the lower limit of the O content is not limited, from the standpoint of the manufacturing cost, in the present disclosure, the O content may be 0.0001% or more. On the other hand, if the O content is excessive, there are cases in which a coarse oxide is generated, and the toughness and ductility of the steel product and the HAZ deteriorate. From the standpoint of ensuring the toughness and ductility of the steel product and the HAZ, the O content is 0.0100% or less. The O content is preferably 0.0060% or less, or 0.0040% or less.

### (N: 0.0100% or less)

N is an impurity element. Although the lower limit of the N content is not limited, from the standpoint of the manufacturing cost, in the present disclosure, the N content may be 0.0001% or more. From the standpoint of ensuring the properties of the steel product and the toughness of the HAZ, in the present disclosure, the N content is 0.0100% or less. The N content is preferably 0.0050% or less, or 0.0040% or less.

The steel product relating to the present disclosure may contain other elements (optional elements) instead of some of the Fe. The following optional elements are given as examples, but the contents of these elements may be 0%.

In order to improve the strength and toughness, as needed, the steel product relating to the present disclosure may be made to contain one or two or more of the optional elements Cu, Cr, Mo, and B that are described hereinafter and have the effect of improving the hardenability.

### (Cu: 1.50% or less)

Cu is an element that is sometimes mixed into the steel product in the manufacturing process. However, the lower limit value of the Cu content is not limited and may be 0%. Further, Cu has little adverse effect on the weldability and on the toughness of the HAZ, and has the effect of improving the hardenability of steel, and therefore, is an element that improves the strength of the steel product. Thus, in the present disclosure, the Cu content may be 0.01% or more. The Cu content is preferably 0.10% or more. However, from the standpoint of suppressing the occurrence of Cu cracking at the time of hot rolling of the steel product, in the present disclosure, the Cu content is 1.50% or less. The Cu content is preferably 1.00% or less, 0.80% or less, 0.60% or less, or 0.50% or less.

### (Cr: 3.00% or less)

Cr is an element that is sometimes mixed into a steel product in the manufacturing process. However, the lower limit value of the Cr content is not limited, and may be 0%. Further, Cr is also an element that improves the strength of a steel product because it has the effect of increasing the hardenability of the steel. Therefore, in the present disclosure, the Cr content may be 0.01% or more. The Cr content is preferably 0.10% or more. However, from the standpoint of suppressing deterioration in the toughness and weldability of the HAZ, in the present disclosure, the Cr content is 3.00% or less. The Cr content is preferably 2.20% or less, 1.40% or less, or 0.80% or less.

### (Mo: 2.00% or less)

Mo is an element that is sometimes mixed into a steel product in the manufacturing process. However, the lower limit value of the Mo content is not limited, and may be 0%. Further, Mo is also an element that improves the strength of a steel product because it has the effect of increasing the hardenability of the steel. Therefore, in the present disclosure, the Mo content may be 0.01% or more. The Mo content is preferably 0.05% or more, 0.10% or more, 0.20% or more or 0.30% or more. However, from the standpoints of suppressing deterioration in the toughness and weldability of the HAZ, and suppressing an increase in the alloy cost, in the present disclosure, the Mo content is 2.00% or less. The Mo content is preferably 1.20% or less, or 0.80% or less.

### (B: 0.0050% or less)

B is an element that is sometimes mixed into a steel product in the manufacturing process. However, the lower limit value of the B content is not limited, and may be 0%. Further, B is also an element that exhibits a marked effect of increasing the hardenability of steel and improves the strength of a steel product. Therefore, in the present disclosure, the B content may be 0.0003% or more. However, from the standpoint of suppressing deterioration in the surface quality of a steel slab manufactured in continuous casting, in the present disclosure, the B content is 0.0050% or less. The B content is preferably 0.0030% or less, or 0.0020% or less.

In order to improve the strength, as needed, the steel product relating to the present disclosure may be made to contain one or two or more of the optional elements Nb, Ti, and V that are described hereinafter and have the effect of increasing the strength of the steel product by precipitates such as carbides or nitrides.

### (Nb: 0.050% or less)

Nb is an element that is sometimes mixed into a steel product in the manufacturing process. However, the lower limit value of the Nb content is not limited, and may be 0%. Further, Nb is also an element that forms a carbide or a nitride, and has the effect of refining the microstructure, and improves the strength of the steel product. Therefore, in the present disclosure, the Nb content may be 0.001% or more. However, from the standpoint of suppressing deterioration in the toughness and weldability of the HAZ, the Nb content is 0.050% or less. The Nb content is preferably 0.040% or less, or 0.030% or less. In particular, from the standpoint of ensuring the toughness of the steel product after PWHT, the Nb content may be 0.004% or less.

### (Ti: 0.050% or less)

Ti is an element that is sometimes mixed into a steel product in the manufacturing process. However, the lower limit value of the Ti content is not limited, and may be 0%. Further, Ti is also an element that forms a carbide or a nitride, and has the effect of refining the microstructure, and improves the strength of the steel product. Therefore, in the present disclosure, the Ti content may be 0.001% or more. However, from the standpoint of suppressing deterioration in the toughness and weldability of the HAZ, the Ti content is 0.050% or less. The Ti content is preferably 0.040% or less, or 0.030% or less. In particular, from the standpoint of ensuring the toughness of the steel product after PWHT, the Ti content may be 0.004% or less, or 0.002% or less.

### (V: 0.10% or less)

V is an element that is sometimes mixed into a steel product in the manufacturing process. However, the lower limit value of the V content is not limited, and may be 0%. Further, V is also an element that forms a carbide or a nitride, and improves the strength of the steel product. Therefore, in the present disclosure, the V content may be 0.01% or more. However, from the standpoints of suppressing deterioration in the toughness and weldability of the HAZ, and suppressing an increase in the alloy cost, the V content is 0.10% or less. The V content is preferably 0.08% or less, or 0.05% or less.

In order to improve the toughness of the HAZ, as needed, the steel product relating to the present disclosure may be made to contain one or two or more of the optional elements Mg, Ca, and REM that are described hereinafter.

### (Mg: 0.0200% or less)

Mg is an element that is sometimes mixed into a steel product in the manufacturing process. However, the lower limit value of the Mg content is not limited, and may be 0%. Further, Mg is also an element that forms an oxide and improves the toughness of the heat affected zone. Therefore, in the present disclosure, the Mg content may be 0.0003% or more, 0.0006% or more, or 0.0010% or more. On the other hand, if the Mg content is excessive, there are cases in which the Mg forms a coarse oxide and decreases the toughness of the steel. Accordingly, from the standpoint of ensuring the toughness, in the present disclosure, the Mg content is 0.0200% or less. The Mg content is preferably 0.0100% or less, 0.0060% or less, or 0.0040% or less.

### (Ca: 0.0200% or less)

Ca is an element that is sometimes mixed into a steel product in the manufacturing process. However, the lower limit value of the Ca content is not limited, and may be 0%. Further, Ca is also an element that, by spheroidizing the sulfide within the steel product, mitigates the effect of the MnS that decreases the toughness of the steel product and the heat affected zone. Therefore, in the present disclosure, the Ca content may be 0.0003% or more, 0.0006% or more, or 0.0010% or more. On the other hand, if the Ca content is excessive, there are cases in which the Ca forms a coarse oxide and decreases the toughness of the steel. Accordingly, from the standpoint of ensuring the toughness, in the present disclosure, the Ca content is 0.0200% or less. The Ca content is preferably 0.0100% or less, 0.0060% or less, or 0.0040% or less.

### (REM: 0.0200% or less)

Rare earth metal (REM) is a collective term for a total of 17 elements that are the two elements of Sc and Y and fifteen lanthanoid elements such as La, Ce, Nd. The REM content means the total content of the aforementioned 17 elements. REMs are elements that are sometimes mixed into a steel product in the manufacturing process. However, the lower limit value of the REM content is not limited, and may be 0%. Further, REMs are also elements that form oxides and improve the toughness of the heat affected zone. Therefore, in the present disclosure, the REM content may be 0.0003% or more, 0.0006% or more, or 0.0010% or more. On the other hand, if the REM content is excessive, there are cases in which the REMs form coarse oxides and decrease the toughness of the steel. Accordingly, from the standpoint of ensuring the toughness, in the present disclosure, the REM content is 0.0200% or less. The REM content is preferably 0.0100% or less, 0.0060% or less, or 0.0040% or less.

### (Balance: Fe and Impurities)

The balance of the chemical composition of the steel product relating to the present disclosure is iron (Fe) and impurities. Impurities mean components that are mixed due to raw materials such as ore and scrap, and other factors, at the time of industrially manufacturing the steel product.

In addition to the limits on the contents of the respective elements, in the present disclosure, the range of value α is limited as follows.

### (Value α: 5.0 or more and 16.0 or less)

Value α is computed by following formula (1). α = 0.50 × √[C] × (1+0.64[Si]) × (1+4.10[Mn]) × (1+0.27[Cu]) × (1+0.52[Ni]) × (1+2.33[Cr]) × (1+3.14[Mo])

Wherein [C], [Si], [Mn], [Cu], [Ni], [Cr] and [Mo] are the contents (mass%) of C, Si, Mn, Cu, Ni, Cr and Mo in the steel. In a case in which a given element is not contained, zero is substituted in. Note that √[C] has the same meaning as [C]^{1/2}.

In the present disclosure, the range of value α is 5.0 - 16.0. This is an index expressing the hardenability of the steel product. The greater the value α, the more that lower bainite and martensite microstructures having a superior balance of strength and toughness can be formed. When α is in the appropriate range, in the microstructure of the HAZ as well, the ratio of the lower bainite and martensite microstructures having a superior balance of strength and toughness becomes high, and the HAZ toughness also can be ensured. When α is 5.0 or more, the hardenability of the base metal is ensured, and the ratio of the lower bainite and martensite having a favorable balance of strength and toughness increases, and a deterioration in toughness is suppressed. Further, in the microstructure of the HAZ as well, it is easy for the ratio of the lower bainite and martensite to increase, and the HAZ toughness also improves. On the other hand, if value α is 16.0 or less, toughness can be ensured without the strength of the steel product becoming too high. Further, when value α is 16.0 or less, the toughness after PWHT also can be ensured. Moreover, the HAZ toughness also is ensured without the HAZ becoming too hard.

Due to the aforementioned numerical value range relating to value α being satisfied, there can be provided a nickel-containing steel product for low temperatures that has excellent strength and toughness. Value α is preferably 5.5 or more, 6.0 or more, or 7.0 or more. Further, value α is preferably 15.5 or less or 15.0 or less.

### <Microstructure>

The microstructure of the steel product relating to the present disclosure is described next. The microstructure of the region that is 1/4 of the thickness in the thickness direction from the surface of the steel product relating to the present disclosure contains lower bainite and martensite. Further, in addition to lower bainite, upper bainite also may be contained as bainite.

"Bainite" is a collective term for upper bainite and lower bainite. "Upper bainite" is one of or both of upper bainite that contains residual austenite or an MA phase (martensite-austenite mixed phase) between the laths, and upper bainite that contains a carbide between the laths. "Lower bainite" is lath-shaped lower bainite containing a carbide within the laths.

There are four forms of "martensite" that are lath, butterfly, lenticular and plate-shaped, but mainly lath martensite is generated in the components of the present disclosure. Lath martensite is a microstructure that is composed of packets and blocks formed from groups of laths having a specific arrangement, and in which a single austenite grain is divided into plural packets.

### (Total of Area Ratios of Lower Bainite and Martensite: 15.0% or more)

Lower bainite and martensite are hard phases and increase the toughness of the steel product. From the standpoint of ensuring the toughness of the steel product, the area ratio of lower bainite and martensite at the 1/4t portion is 15.0% or more. The area ratio of lower bainite and martensite at the 1/4t portion is preferably 20.0% or more, or 30.0% or more. The total of the area ratio of the lower bainite and the area ratio of the martensite at the 1/4t portion may be 100%.

### (Total of Area Ratios of Upper Bainite, Lower Bainite, and Martensite: 90.0% or more)

From the standpoint of ensuring the strength of the steel product, the total of the area ratios of upper bainite and lower bainite and martensite at the 1/4t portion is 90.0% or more. The total of the area ratios of upper bainite, lower bainite and martensite at the 1/4t portion may be 100%. Further, the upper bainite of the 1/4t portion may be 1.0% or more.

### (Area Ratio of Residual Austinite: less than 1.7%)

From the standpoint of ensuring the toughness of the steel product, the area ratio of the residual austenite of the 1/4t portion is less than 1.7%. The area ratio of the residual austenite of the 1/4t portion is preferably 1.0% or less, and may be 0%. This is thought to be because, in the Ni-containing, steel plate of the present disclosure, the Ni content is lower than conventional 9% Ni steel, and therefore, even if residual austenite were to exist at -110°C, it would be unstable, and, if the steel structure were to incur plastic deformation at the crack tip, the residual austenite would change into martensite due to plasticity-induced martensitic transformation. Thus, the residual austenite at room temperature is made to be less than 1.7% as a volume ratio.

Further, the higher the Ni content, the easier it is for the volume ratio of the residual austenite to increase as well. However, an increase in the Ni content is also not preferable in that it leads to an increase in cost.

Observation of the microstructure of the steel product is carried out by using a sample in which a 1/4t portion of the steel product serves as the observed surface. Two types of samples on which (a) electrolytic polishing or (b) nital etching is carried out are prepared. Each sample of (a) and (b) is measured at three places by the following method, and the average value of the three places is used as the area ratio of the microstructure of that steel product. Note that three of each sample of (a) and (b) may be prepared, and the averages of the respective samples may be computed. Or, three places of one sample of each may be measured in a visual field, and the average of each computed.

By using an electrolytically polished sample that, after mirror finishing by mechanical polishing, is subjected to electrolytic polishing that removes the strained layers arising due to the mechanical polishing, measurement of the total of the area ratios of the upper bainite, lower bainite, martensite and residual austenite is carried out by EBSD. The measurement magnification is 200×, and measurement of a range of 400 µm × 400 µm is carried out at a pitch of 0.4 µm. The measuring is carried out in a state in which the beam diameter of the electron beam is 0.4 µm or less. The confidence index (hereinafter called "CI value") is set to 0.1 or more. The determination of ferrite, and upper bainite, lower bainite and martensite, is carried out by setting the threshold value of the Grain Average Misorientation (hereinafter called "GAM") to 0.5. Note that the GAM value is an index defined in OIM Analysis (EBSD crystal orientation analyzing software manufactured by TSL, United States). The region in which the GAM is 0.5 or less is ferrite. The region in which the GAM exceeds 0.5 is upper bainite, lower bainite, martensite or residual austenite. Because the upper bainite, lower bainite, martensite and residual austenite in the present disclosure are determined by using the GAM of EBSD as the threshold value, not only upper bainite, lower bainite, martensite and residual austenite, but also tempered upper bainite, tempered lower bainite and tempered martensite are included. Comparing the microstructures of direct quenching (DQ) and (DQT) that is carried out thereafter up to tempering (T), although dissolution of the MA and coarsening of carbide occur after tempering, the way of looking at the microstructure does not vary greatly.

Measurement of the area ratio of the upper bainite by SEM observation is carried out by using a nital etched sample. The measurement magnification is 500×, and measurement of a range of 360 µm × 480 µm is carried out. The portion, which has a clear lath structure and at which carbide and MA have formed along the lath boundary, is upper bainite. The microstructure of the region, at which the internal structure of the microstructure is relatively coarse, and the density of carbide is low and both sparse and dense, is upper bainite. An example of the results of discriminating the microstructures is shown in Fig. 1. (A) and (B) are SEM images of the same region of a steel product that is manufactured by DQT and whose value α is 9.9. In (B), the regions surrounded by the white lines are upper bainite (Bu), and the other regions are lower bainite + martensite (B_{L}+M). In the portions identified as upper bainite (Bu), carbides appearing white are sparsely distributed, and regions with varying density are present. On the other hand, at the portions identified as lower bainite + martensite (B_{L}+M), the carbides are densely and uniformly distributed. The total of the area ratios of the lower bainite, martensite and residual austenite is determined by subtracting the area ratio of the upper bainite from the total of the area ratios of the upper bainite, lower bainite, martensite and residual austenite, which were measured as described above. Moreover, the area ratio of the residual austenite is determined by the measuring method described hereinafter, and the total of the area ratios of the lower bainite and martensite is determined by subtracting the area ratio of the residual austenite from the total of the area ratios of the lower bainite, martensite and residual austenite.

### (Area Ratio of Residual Austenite)

The area ratio of the residual austenite is measured by X-ray diffraction. Measurement of the area ratio of the residual austenite is carried out by using a sample at which the region, which is 1/4 of the thickness in the thickness direction from the surface of the steel product (also called "1/4t portion" in the present specification), is the measured area. The sample is a 2-mm thick test piece, and is taken from a position that is 1/4 of the width from a width direction end portion of the steel product, and chemical polishing is carried out thereon, and the sample is used in measuring the volume ratio of the residual austenite by X-ray diffraction using an Mo tube. Quantification is carried out on the basis of the ratios of the integrated intensities of the (200), (211) diffraction peaks of the ferrite phase and the integrated intensities of the (200), (220), (311) diffraction peaks of the austenite phase, and the average values of the six combinations are employed. The integrated intensities of the diffraction peaks are determined by fitting the backgrounds on the basis of the signals before and after the peaks, and subtracting the signal differences. The volume ratio measured by the X-ray diffraction is considered to be the area ratio.

### (Average Crystal Grain Diameter of 1/4t Portion of Steel Product)

In the present disclosure, the average crystal grain diameter (effective crystal grain diameter) of the 1/4t portion of the steel product is preferably 20.0 µm or less. This is because it was learned that, if the average crystal grain diameter of the 1/4t portion of the steel product is 20.0 µm or less, the toughness of the steel product tends to improve even more regardless of whether before or after PWHT. However, the average crystal grain diameter of the 1/4t portion of the steel product may exceed 20.0 µm. The smaller the average crystal grain diameter of the steel product, the more preferable, and therefore, the lower limit value thereof is not limited. Usually, the average crystal grain diameter is 10 µm or more. The effective crystal grain diameter is determined by a weighted average. Effective crystal grain diameter Dₐᵣₑₐ that is determined by a weighted average is calculated by the following formula by using, of the crystal grain diameters that are measured in a 4 mm² region, area Si and grain diameter dᵢ of the ith crystal grain detected at the time of measurement. ${D}_{area} = {ΣS}_{i} \cdot {d}_{i} / {ΣS}_{i}$

### (Aspect Ratio of Prior Austenite Crystal Grains of 1/4t Portion of Steel Product)

The form of the prior austenite crystal grains (called prior austenite grains or prior γ grains upon occasion) of the steel product of the present disclosure may be a form that is flat in the rolling direction. If the prior austenite grains of the region that is 1/4 of the thickness in the thickness direction from the surface of the steel product are made to be flat grains of an aspect ratio of 1.5 or more, an even greater improvement in the toughness of the steel product is possible. This is because, by increasing the grain boundary area by making the prior austenite grains flat, there is a substantial refining of the austenite grains, and this is effective in refining the effective crystal grain diameter. The aspect ratio of prior austenite grains is usually 4.0 or less, and may be 3.5 or less.

On the other hand, from the standpoint of ensuring the homogeneity of the microstructure, the aspect ratio of the prior austenite crystal grains of the 1/4t portion may be less than 1.5. The aspect ratio of the prior austenite crystal grains of the 1/4t portion may be 1.4 or less, or 1.3 or less.

The aspect ratio of the prior austenite crystal grains (hereinafter called prior austenite grains upon occasion) of the steel product is determined as follows. An L cross-section (a cross-section parallel to the rolling direction and the thickness direction of the steel product) of the region that is 1/4 of the thickness in the thickness direction from the surface of the steel product is mirror polished, and corrosion is carried out by a corrosive liquid of a saturated solution base of 2 - 4% picric acid, and the prior austenite grain boundaries of an arbitrary region of 1.0 mm in the rolling direction × 0.5 mm in the thickness direction are made to appear.

Next, the long diameters and short diameters of the individual prior austenite grains are measured, and the aspect ratio of each prior austenite grain is calculated by long diameter ÷ short diameter. The arithmetic mean of the calculated aspect ratios of all of the prior austenite grains is determined as the "aspect ratio of the prior austenite grains". Note that the maximum length of the prior austenite grain is used as the long diameter, and the maximum interval between two lines, which contact the grain and are parallel to the long diameter direction, is used as the short diameter.

### <Mechanical Properties>

The steel product relating to the present disclosure has mechanical properties that are such that the steel product has both strength and low-temperature toughness. In addition to having excellent toughness at -110°C in particular, the steel product can exhibit excellent low-temperature toughness after PWHT as well.

### (Tensile Strength: 615 MPa or more and 930 MPa or less)

In the present disclosure, the tensile strength of the steel product is 615 - 930 MPa. In order to reduce the weight of large welded structures such as transport tanks, a steel product that can ensure strength of a structure even if the thickness is thin is necessary. Because steel products that are selected as steel products to be used in such applications usually are steel products having the aforementioned tensile strength, the steel product relating to the present disclosure also is manufactured to have the aforementioned tensile strength.

### (Yield Ratio)

The yield ratio (YR = [yield strength] / [tensile strength] × 100) of the steel product relating to the present disclosure is not particularly limited and is preferably 90% or less. In a case in which there is no yield point, the yield strength is determined by using 0.2% proof stress.

### (Charpy Impact Absorption Energy at -110°C)

In order to ensure high toughness at low temperatures, the Charpy impact absorption energy at -110°C of the steel product of the present disclosure is preferably 150 J or more. Due to the steel product of the present disclosure having low-temperature toughness of a Charpy impact absorption energy at -110°C of 150 J or more, a transport tank formed from the steel product of the present disclosure can be suitably used for transporting liquid carbon dioxide for example. The steel product of the present disclosure may have low-temperature toughness of a Charpy impact absorption energy at -110°C of 100 J or more. Note that the Charpy impact absorption energy at -110°C is a numerical value measured by using a sample taken from a position of 1/4 of the thickness.

### (Charpy Absorption Energy at -110°C after PWHT)

There are cases in which PWHT is carried out on the welded portions of cryogenic tanks after being assembled into transport tanks, in order to prevent breakage in advance. At this time, not only the welded portions, but also the base metal portion (also simply called base metal) of the steel product that is not affected by welding are heated. If the time over which the base metal is heated in the temperature range of 425°C or more is long, the toughness of the base metal tends to decrease. In the steel product of the present disclosure, in a case in which PWHT, in which the holding temperature is 600°C, and the holding time is 2 hours, and the rate of temperature increase and the rate of temperature decrease are 55°C/h in the temperature region of 425°C or more, is carried out on the steel product, with regard to the toughness of the portion where the PWHT has been carried out, the Charpy impact absorption energy at -110°C is preferably 150 J or more. The Charpy impact absorption energy at -110°C after PWHT may be 100 J or more. The Charpy impact absorption energy at -110°C after PWHT also is a numerical value measured by using a sample taken from a position of 1/4 of the thickness.

Note that there are cases in which the toughness of the steel product decreases due to PWHT. Although the reason for this is not clear, it is assumed that P (phosphorus) and Mn diffuse at the grain boundaries, and growth or aggregation of inclusions arises within the microstructure, and due thereto, the brittleness decreases and the toughness decreases. A decrease in the toughness due to PWHT is suppressed by limiting the contents of P and Mn and making the average crystal grain diameter of the steel product small.

### (Charpy Impact Absorption Energy at -110°C after Thermal Cycling)

In the steel product of the present disclosure, in order to ensure high toughness after a thermal cycling test that simulates the welded portions at a low temperature, the Charpy impact absorption energy at -110°C after thermal cycling is preferably 50 J or more. Due to the steel product of the present disclosure having low-temperature toughness that is such that the Charpy impact absorption energy at -110°C after thermal cycling is 50 J or more, a transport tank formed from the steel product of the present disclosure can be suitably used for transporting liquid carbon dioxide for example. The Charpy impact absorption energy at -110°C after thermal cycling may be 40 J or more. Note that the Charpy impact absorption energy at -110°C after thermal cycling is a numerical value measured by using a sample taken from a position of 1/4 of the thickness of the steel product as a thermal cycling test piece, and providing it with a thermal history of raising the temperature at 60°C/s to 1350°C, and, after maintenance at 1350°C for 1 s, cooling at 20°C/s to room temperature, and thereafter, taking a Charpy test piece therefrom.

### (Charpy Impact Absorption Energy at -110°C after Thermal Cycling and PWHT)

There are cases in which PWHT is carried out on the welded portions of cryogenic tanks after being assembled into transport tanks, in order to prevent breakage in advance. After the above-described thermal cycling test, PWHT, in which the rate of temperature increase and the rate of temperature decrease are 55°C/h in the temperature region of 425°C or more, and the steel product is held for 2 hours at 600°C, is carried out on the steel product of the present disclosure, and thereafter, a Charpy test piece is taken, and measurement is carried out. In this case, with regard to the toughness of the portion where the PWHT has been carried out, the Charpy impact absorption energy at -110°C is preferably 50 J or more. The Charpy impact absorption energy at -110°C of the portion at which PWHT is carried out after the above-described thermal cycling test may be 40 J or more.

Note that there are cases in which the toughness of the steel product decreases due to PWHT. Although the reason for this is not clear, it is assumed that P (phosphorus) and Mn diffuse at the grain boundaries, and growth or aggregation of inclusions arises within the microstructure, and due thereto, the brittleness decreases and the toughness decreases. A decrease in the toughness due to PWHT is suppressed by limiting the contents of P and Mn and making the average crystal grain diameter of the steel product small.

The tensile strength (TS) and the yield strength (YS) are measured in accordance with a tensile test that is based on JIS Z2241:2011. The tensile test uses a JIS14A test piece that has been taken from a position of 1/4 of the thickness and whose length direction is the direction (the C direction) parallel to the width direction of the steel product. TS and YS are computed by using three test pieces and taking the averages thereof. The yield ratio (YR, %) is computed by (YS/TS) × 100, on the basis of the respective average values of TS and YS.

The Charpy impact absorption energy is measured by a Charpy impact test at -110°C on the basis of the prescriptions of JIS Z2242:2018 and by using an impact blade of a radius of 2 mm. The Charpy impact absorption energy is calculated by measuring by using three test pieces, and taking the average thereof. The Charpy impact absorption energy test uses a V-notched test piece that has been taken from a position of 1/4 of the thickness of the steel product and whose length direction is the direction (the C direction) parallel to the width direction of the steel product.

The form of the steel product relating to the present disclosure is not particularly limited, and examples are steel plates, steel strips, structural steel and steel pipes. However, steel pipes and structural steel include steel products in which steel plates are joined, e.g., in addition to welded steel pipes and welded structural steel, structural steel joined by rivets, and the like. The thickness of the steel product such as steel plates, steel strips, structural steel and steel pipes (the thickness of the flanges in the case of structural steel) is not particularly limited, and usually is 3 mm or more and 150 mm or less. The thickness of the steel product may be 6 mm or more, 10 mm or more, 15 mm or more, or 30 mm or more. Further, the thickness of the steel product may be 100 mm or less, 80 mm or less, or 60 mm or less.

Further, although the application of the steel product relating to the present disclosure also is not particularly limited, the steel product relating to the present disclosure has mechanical properties such that the steel product has both strength and low-temperature toughness, and, in particular, can exhibit excellent low-temperature toughness even after PWHT. Therefore, the steel product relating to the present disclosure can be suitably used as a tank that stores and transports liquefied gasses, and liquid carbon dioxide in particular.

### (Method of Manufacturing Steel Product)

The method of manufacturing the steel product relating to the present disclosure is not particularly limited, but, for example, after melting a steel that satisfies the above-described chemical composition, a steel slab is manufactured by continuous casting. The steel slab is subjected to either direct quenching (DQ), in which it is heated, hot rolled, and then directly water-cooled, or reheat quenching (RQ), in which it is hot rolled, air-cooled, reheated, and then water-cooled, to made into a steel product. Note that, in the case of RQ, the hot rolled steel does not necessarily have to be air-cooled before reheating, but water cooling may be used.
Moreover, tempering (T) may also be carried out.
(1) DQT: direct quenching (DQ) and tempering (T)
(2) RQT: air cooling or water cooling, reheat quenching (RQ), and tempering (T)

### (1) DQT

From the standpoint of the manufacturing cost, DQT is preferable in the manufacturing of the steel product relating to the present disclosure. An example of a preferable manufacturing process is given hereinafter.

In the case of manufacturing the steel product relating to the present disclosure by DQ, from the standpoint of carrying out hot rolling in a temperature range in which the microstructure of the rolled steel is austenite, the heating temperature of the steel slab on which the hot rolling is carried out is Ac₃ or more. From the standpoint of decreasing the deformation resistance, the heating temperature of the steel slab is preferably 1000°C or more. On the other hand, from the standpoint of suppressing coarsening of the heated γ grains, the heating temperature of the hot rolling is 1250°C or less. The heating temperature of the hot rolling is preferably 1200°C or less. Note that Ac₃ is a value computed by the following formula. Ac3 = 937.2 - 436.5C + 56Si - 19.7Mn - 16.3Cu - 26.6Ni - 4.9Cr + 38.1Mo + 124.8V + 136.3Ti - 19.1Nb + 198.4Al + 3315B

The element symbols in the formula mean the content (mass%) of each element contained in the steel slab.

There are cases in which the hot rolling is structured by rolling in a temperature range in which recrystallization occurs (rolling in the recrystallization temperature range) and rolling in a temperature range in which recrystallization is suppressed (rolling in the non-recrystallization temperature range).

Rolling in the recrystallization temperature range is hot rolling carried out with the temperature of the rolled steel during rolling being 900°C or more. From the standpoint of refining the austenite grain diameter of the steel product, the cumulative rolling reduction ratio of the rolling in the recrystallization temperature range is preferably 20% or more, and more preferably 30% or more. The cumulative rolling reduction ratio of the rolling in the recrystallization temperature range is determined from the difference between the thickness of the steel slab before hot rolling and the thickness of the rolled steel at 900°C. Cumulative rolling reduction ratio (%) of rolling in recrystallization temperature range = 100 × ([thickness of steel slab] - [thickness of rolled steel at 900°C]) / [thickness of steel slab]

Rolling in the non-recrystallization temperature range is hot rolling carried out with the temperature of the rolled steel during rolling being less than 900°C. From the standpoint of refining the average crystal grain diameter of the steel product, the cumulative rolling reduction ratio of the rolling in the non-recrystallization temperature range is preferably 20% or more, and more preferably 30% or more. The cumulative rolling reduction ratio of the rolling in the non-recrystallization temperature range is determined from the difference between the thickness of the rolled steel at 900°C and the thickness of the steel product after rolling ends. Cumulative rolling reduction ratio (%) of rolling in non-recrystallization temperature range = 100 × ([thickness of rolled steel at 900°C] - [thickness of steel product after rolling ends]) / [thickness of rolled steel at 900°C]

From the standpoint of suppressing the generation of ferrite that decreases strength, the end temperature of the hot rolling is Ar₃ or more. After hot rolling ends, accelerated cooling such as water cooling is carried out on the steel product. From the standpoint of suppressing the generation of ferrite that decreases strength, the start temperature of the accelerated cooling is Ar₃ or more. Note that Ar₃ is a value computed by the following formula. ${Ar}_{3} = 910 - 310 C - 80 Mn - 20 Cu - 15 Cr - 55 Ni - 80 Mo + 0.35 \left(t-8\right)$

The element symbols in the formula mean the content (mass%) of each element contained in the steel product, and t means the thickness (mm) of the steel product.

From the standpoint of promoting bainitic transformation and martensitic transformation, the cooling rate is 1.0°C/s or more. The cooling rate of the accelerated cooling is preferably 5.0°C/s or more, or 10.0°C/s or more. The faster the cooling rate of the accelerated cooling, the more preferable, but from standpoints such as cost and homogeneity of the accelerated cooling, the cooling rate is preferably 50.0°C/s or less, or 30.0°C/s or less. The cooling rate is a value obtained by calculating the cooling rate at a position of 1/4 of the thickness by simulation in accordance with thermal transfer calculation.

From the standpoint of improving the strength of the steel product by ensuring the upper bainite, lower bainite and martensite, the stoppage temperature of the accelerated cooling is 400°C or less. The stoppage temperature of the accelerated cooling is preferably 350°C or less. Accelerated cooling may be carried out to room temperature. From the standpoint of dehydrogenation of the steel product, the stoppage temperature is preferably 100°C or more.

After accelerated cooling, a tempering treatment may be carried out on the steel product. From the standpoint of suppressing a decrease in strength, the heating temperature of the tempering treatment is preferably 650°C or less, 620°C or less, or 590°C or less. On the other hand, from the standpoint of improving the toughness, the heating temperature of the tempering treatment is preferably 350°C or more, or 400°C or more.

### (2) RQT

In a case in which the steel product relating to the present disclosure is manufactured by RQ, the effects of the heating temperature and the rolling reduction ratio of the steel slab at the time of the hot rolling on the mechanical properties of the steel product are small. However, if the heating temperature of the steel slab is too low, the deformation resistance increases, and therefore, the heating temperature of the steel slab is preferably 1000°C or more. Further, if the rolling reduction ratio is insufficient, there are cases in which initial stage defects from the time of manufacturing the steel slab remain at the thickness central portion, and the quality of the steel product decreases. Therefore, the total of the rolling reduction ratios of hot rolling (also called cumulative rolling reduction ratio) is preferably 35% or more. After the hot rolling, the steel slab may, as is, be water-cooled or air-cooled.

After the hot rolling, reheat quenching is carried out on the steel product. The reheating temperature of the steel product is Ac₃ or more, because quenching is carried out from an austenite single-phase microstructure. From the standpoint of ensuring the homogeneity of the microstructure, the reheating temperature of the steel product is preferably 750°C or more, 850°C or more, 880°C or more, or 900°C or more. On the other hand, although the upper limit temperature of the reheating temperature is not particularly stipulated, there are cases in which excessive heating to a high temperature leads to coarsening of the austenite grains and a decrease in toughness, and therefore, the upper limit temperature of the reheating temperature is preferably 1000°C or less, 950°C or less, or 930°C or less.

After the reheat quenching, a tempering treatment may be carried out on the steel product. From the standpoint of suppressing a decrease in strength, the heating temperature of the tempering treatment is preferably 660°C or less, or 640°C or less. On the other hand, from the standpoint of improving the toughness, the heating temperature of the tempering treatment is preferably 400°C or more, 450°C or more, or 500°C or more.

### EXAMPLES

The steel product relating to the present disclosure is described concretely hereinafter by way of Examples. However, the conditions in the following Examples are examples of conditions that are employed in order to confirm the feasibility and the effects of the present disclosure, and the present disclosure is not limited to the following Examples.

### <Manufacturing by Direct Quenching and Tempering>

### [Manufacturing of Steel Product]

First, slabs having the chemical compositions shown in Table 1 were cast by continuous casting. The balance, which is other than the components listed in Table 1, is Fe and impurities. Further, blank cells mean that the alloy elements were not intentionally added in the steelmaking process. The underlines mean that the value is outside of the scope of the present disclosure.

**[Table 1]**

| No. | chemical composition (mass%) | | | | | | | | | | | | | | | | | | | |
|---|---|---|---|---|---|---|---|---|---|---|---|---|---|---|---|---|---|---|---|---|
| | C | Si | Mn | P | S | Ni | Al | N | O | Ti | Nb | Mg | Ca | REM | Cu | Cr | Mo | V | B | α |
| 2A | 0.14 | 0.14 | 1.81 | 0.011 | 0.0060 | 5.95 | 0.033 | 0.0019 | 0.0022 | | | | | | | | | | | 7.0 |
| 3A | 0.14 | 0.18 | 1.45 | 0.012 | 0.0071 | 5.52 | 0.030 | 0.0021 | 0.0024 | 0.004 | 0.004 | | | | | | | 0.06 | | 5.6 |
| 4A | 0.11 | 0.19 | 1.47 | 0.004 | 0.0041 | 5.73 | 0.005 | 0.0018 | 0.0025 | 0.002 | | | 0.0013 | | | | | 0.04 | | 5.2 |
| 6A | 0.06 | 0.13 | 0.66 | 0.006 | 0.0029 | 5.88 | 0.036 | 0.0073 | 0.0018 | 0.001 | 0.003 | | | | 0.56 | 0.42 | 0.15 | | | 6.7 |
| 7A | 0.06 | 0.18 | 1.07 | 0.006 | 0.0024 | 5.62 | 0.029 | 0.0021 | 0.0015 | | | | | | | 0.22 | 0.18 | | 0.0003 | 6.8 |
| 8A | 0.15 | 0.26 | 1.20 | 0.008 | 0.0021 | 5.88 | 0.026 | 0.0027 | 0.0019 | | | 0.0023 | | | 0.20 | | 0.11 | | | 7.7 |
| 9A | 0.17 | 0.22 | 1.40 | 0.007 | 0.0027 | 5.90 | 0.020 | 0.0030 | 0.0022 | | | | | | 0.15 | | 0.05 | | | 7.8 |
| 10A | 0.08 | 0.13 | 0.62 | 0.005 | 0.0015 | 5.52 | 0.029 | 0.0019 | 0.0036 | | | | | | 0.47 | 0.20 | 0.51 | | 0.0005 | 9.0 |
| 11A | 0.12 | 0.15 | 0.80 | 0.005 | 0.0026 | 5.27 | 0.034 | 0.0071 | 0.0041 | | | | 0.0014 | 0.0011 | 0.60 | 0.76 | | | | 9.8 |
| 12A | 0.10 | 0.12 | 0.75 | 0.006 | 0.0019 | 5.71 | 0.055 | 0.0039 | 0.0022 | 0.002 | | 0.0014 | | | | 0.32 | 0.43 | 0.02 | | 11.3 |
| 13A | 0.07 | 0.17 | 0.73 | 0.006 | 0.0032 | 5.44 | 0.046 | 0.0043 | 0.0028 | | 0.002 | | | | | 0.54 | 0.46 | | | 12.4 |
| 14A | 0.08 | 0.13 | 0.98 | 0.011 | 0.0116 | 5.21 | 0.056 | 0.0021 | 0.0015 | | | | | | 0.65 | 0.43 | 0.25 | | | 12.0 |
| 15A | 0.06 | 0.17 | 0.73 | 0.009 | 0.0032 | 5.44 | 0.046 | 0.0043 | 0.0028 | 0.002 | | | | | 0.33 | 0.43 | 0.52 | 0.02 | | 11.9 |
| 16A | 0.05 | 0.13 | 1.15 | 0.008 | 0.0075 | 5.35 | 0.034 | 0.0025 | 0.0019 | | 0.002 | | 0.0010 | | 0.44 | 0.39 | 0.33 | | | 11.4 |
| 17A | 0.11 | 0.12 | 1.28 | 0.007 | 0.0053 | 5.83 | 0.006 | 0.0063 | 0.0019 | | | | | | 0.40 | 0.43 | 0.10 | | | 13.1 |
| 19A | 0.07 | 0.06 | 1.31 | 0.009 | 0.0044 | 5.11 | 0.038 | 0.0038 | 0.0027 | | 0.003 | | | 0.0012 | | | 1.03 | | | 13.6 |
| 20A | 0.09 | 0.11 | 0.85 | 0.010 | 0.0065 | 5.33 | 0.029 | 0.0031 | 0.0015 | | | | | | 0.43 | 0.71 | 0.22 | | | 13.6 |
| 21A | 0.11 | 0.07 | 1.26 | 0.007 | 0.0038 | 5.30 | 0.035 | 0.0035 | 0.0022 | 0.003 | | | | | | 0.44 | 0.22 | | | 13.7 |
| 22A | 0.08 | 0.13 | 0.80 | 0.006 | 0.0056 | 5.12 | 0.025 | 0.0028 | 0.0017 | | 0.002 | 0.0013 | | | 0.43 | 0.71 | 0.35 | | | 14.9 |
| 24A | 0.14 | 0.14 | 1.69 | 0.013 | 0.0064 | 5.85 | 0.029 | 0.0020 | 0.0019 | | 0.003 | | | | | | | | | 6.5 |
| 25A | 0.05 | 0.05 | 0.33 | 0.008 | 0.0018 | 5.80 | 0.006 | 0.0028 | 0.0021 | | | | | | | 1.63 | | | 0.0011 | 5.2 |
| 26A | 0.10 | 0.19 | 1.12 | 0.014 | 0.0008 | 5.44 | 0.029 | 0.0048 | 0.0029 | 0.002 | 0.003 | 0.0020 | 0.0014 | | | | 0.74 | | | 12.6 |
| 28A | 0.15 | 0.07 | 1.80 | 0.012 | 0.0019 | 5.25 | 0.074 | 0.0034 | 0.0023 | | | | | | 0.15 | 0.23 | 0.25 | | | 18.0 |
| 30A | 0.06 | 0.13 | 1.45 | 0.007 | 0.0051 | 6.34 | 0.025 | 0.0028 | 0.0017 | | 0.002 | 0.0010 | | | 0.43 | 0.71 | 0.35 | | | 24.6 |
| 31A | 0.05 | 0.12 | 2.43 | 0.013 | 0.0009 | 5.30 | 0.028 | 0.0023 | 0.0019 | | | | | | 0.10 | 0.15 | 0.27 | | | 12.7 |
| 32A | 0.10 | 0.13 | 0.87 | 0.008 | 0.0022 | 4.98 | 0.022 | 0.0031 | 0.0033 | | | | | 0.0012 | 0.22 | 0.42 | 0.29 | 0.02 | | 11.2 |
| 101A | 0.08 | 0.05 | 1.32 | 0.014 | 0.0036 | 4.78 | 0.004 | 0.0021 | 0.0033 | 0.011 | | | | | 0.20 | | 0.28 | 0.03 | | 6.5 |
| 102A | 0.14 | 0.08 | 1.41 | 0.008 | 0.0041 | 5.45 | 0.032 | 0.0018 | 0.0024 | | | | | | | | | | | 5.1 |
| 103A | 0.11 | 0.15 | 1.50 | 0.009 | 0.0053 | 5.11 | 0.034 | 0.0032 | 0.0019 | 0.008 | 0.023 | 0.0061 | | | | | 0.23 | | | 8.2 |
| 104A | 0.08 | 0.09 | 1.34 | 0.007 | 0.0022 | 4.91 | 0.027 | 0.0024 | 0.0018 | | | | 0.0046 | | 0.40 | 0.36 | 0.25 | | | 12.6 |
| 105A | 0.09 | 0.07 | 1.22 | 0.005 | 0.0037 | 5.47 | 0.032 | 0.0031 | 0.0036 | 0.014 | | | | | 0.23 | 0.23 | 0.31 | | | 11.6 |
| 106A | 0.11 | 0.05 | 0.95 | 0.006 | 0.0018 | 5.87 | 0.025 | 0.0039 | 0.0027 | | | | | 0.0044 | 0.45 | 0.17 | 0.42 | | 0.0010 | 12.3 |
| 107A | 0.10 | 0.15 | 0.89 | 0.007 | 0.0023 | 5.05 | 0.031 | 0.0041 | 0.0025 | | | | | | 0.28 | 0.33 | 0.46 | | | 13.6 |
| 108A | 0.08 | 0.11 | 1.17 | 0.008 | 0.0016 | 5.35 | 0.028 | 0.0024 | 0.0034 | 0.009 | | | | | 0.35 | 0.46 | 0.34 | | | 15.6 |
| 109A | 0.09 | 0.07 | 1.34 | 0.004 | 0.0034 | 5.81 | 0.025 | 0.0019 | 0.0018 | | 0.030 | | | | 0.44 | 0.21 | 0.37 | | | 14.7 |
| 110A | 0.11 | 0.17 | 1.32 | 0.011 | 0.0034 | 5.74 | 0.026 | 0.0027 | 0.0027 | | 0.003 | | | | | 0.32 | | | | 8.2 |
| 111A | 0.08 | 0.17 | 1.50 | 0.006 | 0.0044 | 5.30 | 0.031 | 0.0032 | 0.0022 | | | 0.0005 | | | | | 0.37 | | | 9.1 |
| 112A | 0.07 | 0.08 | 1.22 | 0.007 | 0.0026 | 4.99 | 0.028 | 0.0024 | 0.0017 | | | | 0.0005 | | 0.35 | 0.30 | 0.24 | | | 9.8 |
| 113A | 0.12 | 0.05 | 0.98 | 0.005 | 0.0015 | 5.77 | 0.033 | 0.0039 | 0.0025 | | | | | 0.0005 | 0.40 | 0.10 | 0.36 | | | 10.4 |
| 114A | 0.08 | 0.13 | 1.05 | 0.012 | 0.0036 | 5.21 | 0.033 | 0.0026 | 0.0018 | | | | | | | | 0.03 | | | 3.3 |
| 115A | 0.07 | 0.15 | 1.24 | 0.009 | 0.0028 | 5.46 | 0.029 | 0.0021 | 0.0022 | | | | | | | 0.04 | | | | 3.7 |
| 116A | 0.12 | 0.09 | 1.73 | 0.011 | 0.0025 | 5.67 | 0.032 | 0.0028 | 0.0028 | | | | | | 0.13 | 0.25 | 0.26 | | | 17.4 |
| 117A | 0.17 | 0.12 | 1.89 | 0.014 | 0.0028 | 5.43 | 0.034 | 0.0031 | 0.0022 | | | | | | 0.17 | 0.23 | 0.17 | | | 18.3 |
| 118A | 0.08 | 0.11 | 1.32 | 0.006 | 0.0051 | 5.12 | 0.033 | 0.0025 | 0.0026 | | 0.004 | | | | | 0.19 | | | | 5.1 |

Next, steel products were manufactured from these slabs under the manufacturing conditions listed in Table 2. "Temper heat treatment" is the heating temperature in the tempering treatment after the quenching.

**[Table 2]**

| No. | plate thickness (mm) | Ac₃ [°C] | hot rolling conditions | | | | | Ar₃ [°C] | direct quenching (accelerated cooling) conditions | | | Temper heat treatment [°C] |
|---|---|---|---|---|---|---|---|---|---|---|---|---|
| | | | heating temperature [°C] | cumulative rolling reduction [%] ratio at 900°C or more | cumulative rolling reduction ratio [%] at less than 900°C | end temperature [°C] | cooling after rolling | | start temperature [°C] | stoppage temperature [°C] | **cooling** rate [°C/s] | |
| 2A | 35 | 697 | 1230 | 23 | 60 | 820 | water cooling | 404 | 800 | 180 | 9.5 | 510 |
| 3A | 25 | 725 | 1150 | 30 | 50 | 810 | water cooling | 453 | 800 | 160 | 5.3 | 540 |
| 4A | 15 | 725 | 1150 | 31 | 59 | 790 | water cooling | 446 | 770 | 150 | 5.7 | 640 |
| 6A | 35 | 751 | 1130 | 31 | 45 | 770 | water cooling | 495 | 750 | 270 | 12.2 | 610 |
| 7A | 60 | 763 | 1170 | 32 | 30 | 780 | water cooling | 497 | 760 | 290 | 2.9 | 600 |
| 8A | 40 | 712 | 1200 | 19 | 65 | 810 | water cooling | 443 | 790 | 250 | 3.1 | 610 |
| 9A | 20 | 694 | 1100 | 22 | 43 | 775 | water cooling | 418 | 750 | 220 | 4.1 | 590 |
| 10A | 35 | 769 | 1240 | 34 | 44 | 750 | water cooling | 488 | 720 | 115 | 3.3 | 580 |
| 11A | 20 | 731 | 1150 | 38 | 45 | 730 | water cooling | 500 | 715 | 320 | 4.2 | 510 |
| 12A | 50 | 762 | 1020 | 39 | 33 | 820 | water cooling | 480 | 800 | 360 | 2.7 | 570 |
| 13A | 55 | 781 | 1080 | 42 | 31 | 770 | water cooling | 502 | 745 | 220 | 10.7 | 610 |
| 14A | 60 | 760 | 1070 | 37 | 38 | 740 | water cooling | 499 | 710 | 240 | 3.7 | 620 |
| 15A | 40 | 786 | 1200 | 25 | 45 | 740 | water cooling | 490 | 722 | 320 | 4.5 | 605 |
| 16A | 55 | 768 | 1100 | 44 | 37 | 760 | water cooling | 484 | 748 | 180 | 6.3 | 560 |
| 17A | 50 | 712 | 1160 | 32 | 29 | 820 | water cooling | 445 | 800 | 210 | 4.2 | 530 |
| 19A | 55 | 795 | 1080 | 33 | 38 | 760 | water cooling | 437 | 725 | 290 | 5.4 | 560 |
| 20A | 50 | 749 | 1100 | 36 | 31 | 840 | water cooling | 499 | 815 | 105 | 2.2 | 480 |
| 21A | 35 | 741 | 1200 | 38 | 50 | 800 | water cooling | 469 | 784 | 243 | 2.9 | 490 |
| 22A | 40 | 765 | 1100 | 30 | 40 | 790 | water cooling | 504 | 779 | 219 | 3.6 | 590 |
| 24A | 57 | 701 | 1200 | 35 | 13 | 780 | water cooling | 427 | 756 | 320 | 5.4 | 490 |
| 25A | 55 | 754 | 1130 | 12 | 35 | 790 | water cooling | 541 | 778 | 290 | 7.8 | 460 |
| 26A | 60 | 772 | 1200 | 32 | 11 | 740 | water cooling | 449 | 730 | 240 | 4.6 | 560 |
| 28A | 55 | 721 | 1120 | 33 | 36 | 720 | water cooling | 421 | 700 | 270 | 4.3 | 550 |
| 30A | 40 | 729 | 1150 | 35 | 38 | 750 | water cooling | 391 | 730 | 220 | 7.4 | 560 |
| 31A | 61 | 747 | 1200 | 32 | 41 | 780 | water cooling | 401 | 753 | 227 | 4.1 | 550 |
| 32A | 50 | 763 | 1100 | 28 | 29 | 840 | water cooling | 516 | 820 | 105 | 0.5 | 490 |
| 101A | 50 | 765 | 1150 | 58 | 60 | 810 | water cooling | 505 | 790 | 310 | 12.5 | 510 |
| 102A | 40 | 714 | 1200 | 60 | 60 | 820 | water cooling | 465 | 800 | 283 | 13.1 | 460 |
| 103A | 70 | 748 | 1100 | 50 | 53 | 790 | water cooling | 478 | 778 | 216 | 7.9 | 610 |
| 104A | 53 | 757 | 1170 | 60 | 56 | 780 | water cooling | 490 | 764 | 189 | 15.2 | 550 |
| 105A | 45 | 747 | 1150 | 55 | 58 | 790 | water cooling | 464 | 768 | 223 | 10.5 | 420 |
| 106A | 40 | 733 | 1200 | 58 | 67 | 810 | water cooling | 443 | 792 | 196 | 6.9 | 580 |
| 107A | 50 | 768 | 1100 | 49 | 59 | 770 | water cooling | 497 | 746 | 143 | 7.9 | 480 |
| 108A | 55 | 755 | 1070 | 60 | 54 | 790 | water cooling | 473 | 774 | 178 | 15.7 | 500 |
| 109A | 48 | 731 | 1200 | 56 | 63 | 800 | water cooling | 428 | 769 | 221 | 18.3 | 530 |
| 110A | 57 | 724 | 1200 | 12 | 56 | 810 | water cooling | 467 | 788 | 343 | 14.2 | 470 |
| 111A | 55 | 762 | 1200 | 55 | 58 | 810 | water cooling | 461 | 793 | 230 | 10.2 | 530 |
| 112A | 45 | 762 | 1100 | 55 | 61 | 820 | water cooling | 499 | 806 | 312 | 12.5 | 420 |
| 113A | 65 | 728 | 1150 | 52 | 55 | 790 | water cooling | 459 | 776 | 187 | 6.8 | 620 |
| 114A | 40 | 758 | 1200 | 43 | 40 | 780 | water cooling | 523 | 765 | 253 | 12.1 | 580 |
| 115A | 50 | 751 | 1100 | 37 | 45 | 790 | water cooling | 503 | 778 | 344 | 10.9 | 470 |
| 116A | 55 | 718 | 1150 | 60 | 50 | 810 | water cooling | 412 | 722 | 293 | 8.4 | 580 |
| 117A | 60 | 697 | 1050 | 50 | 40 | 800 | water cooling | 405 | 740 | 365 | 9.8 | 560 |
| 118A | 40 | 752 | 1100 | 39 | 45 | 780 | water cooling | 506 | 430 | 341 | 9.8 | 520 |

### [Measurement and Evaluation]

The microstructures and mechanical properties of the obtained steel products were measured by the above-described methods. The results are shown in Table 3. The meanings of the symbols of the microstructures are as follows. Note that the remainders of the microstructures were pearlite, MA phase, and ferrite.
Bu: upper bainite
BL: lower bainite
M: martensite
residual y: residual austenite

For the toughness, the average value of the Charpy impact absorption energy at -110°C, and the average value of the Charpy impact absorption energy at -110°C after PWHT in which the holding temperature was 600°C, the holding time was 2 hours, and the rate of temperature increase and the rate of temperature decrease in the temperature region of 425°C or more were 55°C/h, respectively were measured.

**[Table 3]**

| No. | microstructure (area ratio) | | | aspect ratio average value of prior γ grains | average crystal grain diameter [µm] | YS [MPa] | TS [MPa] | YR [%] | base metal toughness KV2[J] | toughness after PWHT KV2[J] | thermal cycling toughness KV2[J] | toughness after thermal cycling and PWHT KV2 [J] | notes |
|---|---|---|---|---|---|---|---|---|---|---|---|---|---|
| | BL+M [%] | Bu+BL+M [%] | residual γ [%] | | | | | | | | | | |
| 2A | 27.4 | 92.3 | 0.1 | 2.9 | 22.6 | 564 | 643 | 88 | 189 | 151 | | | examples of present invention |
| 3A | 22.4 | 92.6 | 0.0 | 2.8 | 17.1 | 534 | 623 | 86 | 239 | 196 | | | |
| 4A | 22.8 | 94.1 | 0.1 | 2.6 | 16.7 | 510 | 624 | 82 | 239 | 221 | | | |
| 6A | 35.1 | 92.4 | 0.2 | 3.1 | 17.4 | 568 | 653 | 87 | 243 | 225 | | | |
| 7A | 35.7 | 92.8 | 0.3 | 3.3 | 15.6 | 563 | 661 | 85 | 312 | 319 | | | |
| 8A | 33.1 | 92.1 | 0.2 | 3.0 | 23.9 | 582 | 672 | 87 | 189 | 188 | | | |
| 9A | 38.4 | 94.3 | 0.2 | 3.2 | 21.6 | 576 | 678 | 85 | 179 | 180 | | | |
| 10A | 50.8 | 94.3 | 0.5 | 2.8 | 13.3 | 615 | 729 | 84 | 288 | 285 | | | |
| 11A | 55.1 | 95.2 | 0.4 | 2.7 | 14.8 | 631 | 765 | 82 | 282 | 280 | | | |
| 12A | 65.9 | 93.4 | 0.7 | 3.2 | 12.4 | 659 | 774 | 85 | 285 | 268 | | | |
| 13A | 68.3 | 96.1 | 0.4 | 3.4 | 11.3 | 661 | 759 | 87 | 312 | 297 | | | |
| 14A | 65.4 | 93.9 | 0.5 | 3.2 | 16.5 | 668 | 752 | 89 | 228 | 222 | | | |
| 15A | 64.2 | 95.8 | 0.4 | 3.1 | 15.3 | 665 | 765 | 87 | 242 | 221 | | | |
| 16A | 61.9 | 95.1 | 0.3 | 3.0 | 17.1 | 658 | 748 | 88 | 229 | 211 | | | |
| 17A | 91.7 | 96.0 | 0.6 | 3.1 | 17.4 | 723 | 834 | 87 | 242 | 239 | | | |
| 19A | 98.1 | 98.1 | 0.7 | 3.0 | 17.9 | 715 | 834 | 86 | 252 | 234 | | | |
| 20A | 93.2 | 96.3 | 0.8 | 2.9 | 18.3 | 780 | 910 | 86 | 210 | 208 | | | |
| 21A | 94.4 | 98.1 | 0.5 | 2.8 | 15.6 | 723 | 845 | 86 | 242 | 221 | | | |
| 22A | 92.5 | 96.8 | 0.7 | 2.7 | 14.3 | 754 | 866 | 87 | 253 | 234 | | | |
| 24A | 81.9 | 91.2 | 0.4 | 1.5 | **27.4** | 534 | 645 | 83 | 143 | 101 | | | |
| 25A | 46.3 | 93.0 | 0.3 | 3.2 | **28.7** | 534 | 673 | 79 | 140 | 138 | | | |
| 26A | 82.1 | 91.2 | 0.4 | 1.5 | **27.5** | 664 | 787 | 84 | 146 | 107 | | | |
| 28A | 96.4 | 98.1 | 1.5 | 2.6 | 16.3 | 881 | **991** | 89 | 156 | 121 | | | comparative example |
| 30A | 95.4 | 97.1 | **1.9** | 2.9 | 17.8 | 912 | **1049** | 87 | **112** | **98** | | | |
| 31A | 89.1 | 93.4 | 0.3 | 2.8 | 18.3 | 743 | 865 | 86 | 156 | **34** | | | |
| 32A | **9.3** | 91.3 | 0.1 | 2.7 | 17.6 | 520 | 654 | 80 | **31** | **25** | | | |
| 101A | 33.2 | 92.9 | 0.3 | 3.3 | 16.2 | 571 | 662 | 86 | 248 | 210 | 138 | 126 | examples of present invention |
| 102A | 23.9 | 93.8 | 0.2 | 3.4 | 16.1 | 583 | 657 | 89 | 238 | 231 | 135 | 133 | |
| 103A | 40.3 | 92.2 | 0.3 | 3.2 | 16.6 | 569 | 671 | 85 | 228 | 196 | 142 | 122 | |
| 104A | 62.1 | 96.1 | 0.5 | 3.6 | 13.8 | 663 | 753 | 88 | 286 | 279 | 173 | 171 | |
| 105A | 65.4 | 95.4 | 0.4 | 3.2 | 13.4 | 671 | 759 | 88 | 276 | 245 | 188 | 171 | |
| 106A | 63.7 | 97.2 | 0.6 | 3.4 | 12.2 | 669 | 770 | 87 | 271 | 268 | 179 | 176 | |
| 107A | 92.2 | 96.9 | 1.1 | 3.0 | 15.8 | 753 | 852 | 88 | 249 | 243 | 164 | 167 | |
| 108A | 98.3 | 98.3 | 0.9 | 3.4 | 14.8 | 746 | 864 | 86 | 253 | 228 | 157 | 138 | |
| 109A | 95.4 | 98.2 | 0.8 | 3.3 | 15.1 | 751 | 870 | 86 | 244 | 216 | 161 | 145 | |
| 110A | 39.1 | 93.1 | 0.4 | 2.7 | 27.1 | 585 | 673 | 87 | 133 | 105 | 145 | 128 | |
| 111A | 53.4 | 94.0 | 0.5 | 2.8 | 13.2 | 618 | 734 | 84 | 288 | 285 | 177 | 175 | |
| 112A | 56.8 | 95.2 | 0.4 | 2.7 | 12.2 | 632 | 764 | 83 | 282 | 280 | 183 | 182 | |
| 113A | 63.2 | 95.1 | 0.5 | 2.8 | 12.0 | 639 | 770 | 83 | 288 | 285 | 189 | 188 | |
| 114A | 17.1 | **76.2** | 0.2 | 2.9 | 38.5 | 515 | **588** | 88 | **80** | **75** | **45** | **42** | comparative example |
| 115A | 18.4 | **77.4** | 0.2 | 3.0 | 37.9 | 516 | **590** | 87 | 77 | **74** | **42** | **43** | |
| 116A | 97.2 | 97.9 | 1.2 | 2.8 | 16.1 | 878 | **982** | 89 | 142 | 138 | 39 | 33 | |
| 117A | 96.3 | 98.2 | 1.1 | 2.7 | 15.8 | 880 | **988** | 89 | 138 | 135 | 36 | 32 | |
| 118A | 22.4 | **68.1** | 0.3 | 2.8 | 15.8 | 412 | **523** | 79 | 148 | 133 | 116 | 103 | |

Nos. 2A - 26A, 101A - 113A are Examples of the present invention, and Nos. 28A - 32A, 114A - 118A are Comparative Examples.

In No. 28A, value α exceeded the upper limit value of the present disclosure, and the hardenability was too high, and the strength was excessive.

In No. 30A, value α exceeded the upper limit value of the present disclosure, and the hardenability was too high, and the strength was excessive. Because there was also too much residual γ, sufficient low-temperature toughness was not obtained.

In No. 31A, because Mn fell outside of the upper limit, the low-temperature toughness after PWHT was low.

In No. 32A, because the cooling rate of the direct quenching was low, the total area ratio of the lower bainite and martensite was insufficient, and sufficient low-temperature toughness was not obtained.

In Nos. 114A and 115A, value α was less than the lower limit value of the present disclosure, and the hardenability was insufficient, and the strength was insufficient. Sufficient low-temperature toughness also was not obtained.

In Nos. 116A and 117A, value α exceeded the upper limit value of the present disclosure, and the hardenability was too high, and the strength was excessive.

In No. 118A, the start temperature of the direct quenching was too low, and the total area ratio of the upper bainite, lower bainite and martensite was insufficient, and the strength was insufficient.

In contrast to the Comparative Examples, in the Examples of the present invention, the chemical compositions and microstructures of the steel products were controlled appropriately, and the tensile strengths were in the appropriate range of 615 MPa or more and 930 MPa or less. In addition, low-temperature toughness at -110°C of 100 J or more was obtained regardless of whether before or after PWHT.

### <Manufacturing by Reheat Quenching and Tempering>

### [Manufacturing of Steel Product]

First, slabs having the chemical compositions shown in Table 4 were cast by continuous casting. The balance, which is other than the components listed in Table 4, is Fe and impurities. Further, blank cells mean that the alloy elements were not intentionally added in the steelmaking process. The underlines mean that the value is outside of the scope of the present disclosure.

**[Table 4]**

| No. | chemical composition (mass%) | | | | | | | | | | | | | | | | | | | |
|---|---|---|---|---|---|---|---|---|---|---|---|---|---|---|---|---|---|---|---|---|
| | C | Si | Mn | P | S | Ni | Al | N | O | Ti | Nb | Mg | Ca | REM | Cu | Cr | Mo | V | B | α |
| 2B | 0.13 | 0.13 | 1.86 | 0.010 | 0.0057 | 5.99 | 0.034 | 0.0022 | 0.0024 | | | | | | | | | | | 6.9 |
| 4B | 0.12 | 0.21 | 1.50 | 0.006 | 0.0046 | 5.84 | 0.004 | 0.0015 | 0.0078 | 0.003 | | | 0.0071 | | | | | 0.03 | | 5.7 |
| 6B | 0.05 | 0.11 | 0.72 | 0.005 | 0.0035 | 5.76 | 0.035 | 0.0071 | 0.0017 | 0.002 | 0.004 | | | | 0.49 | 0.44 | 0.12 | | | 6.0 |
| 7B | 0.07 | 0.20 | 1.21 | 0.007 | 0.0019 | 5.69 | 0.028 | 0.0026 | 0.0014 | | | | | | | 0.21 | 0.21 | | 0.0015 | 8.7 |
| 8B | 0.14 | 0.22 | 1.18 | 0.007 | 0.0028 | 5.73 | 0.022 | 0.0031 | 0.0018 | | | 0.0013 | | | 0.23 | | 0.15 | | | 7.7 |
| 9B | 0.18 | 0.24 | 1.37 | 0.005 | 0.0031 | 5.98 | 0.026 | 0.0027 | 0.0025 | | | | | | 0.17 | | 0.08 | | | 8.7 |
| 10B | 0.07 | 0.11 | 0.55 | 0.006 | 0.0022 | 5.31 | 0.022 | 0.0018 | 0.0031 | | | | | | 0.51 | 0.26 | 0.46 | | 0.0004 | 7.7 |
| 11B | 0.14 | 0.14 | 0.76 | 0.008 | 0.0029 | 5.44 | 0.038 | 0.0074 | 0.0044 | | | | 0.0012 | 0.0021 | 0.64 | 0.70 | | | | 9.9 |
| 14B | 0.07 | 0.15 | 0.92 | 0.010 | 0.0122 | 5.38 | 0.052 | 0.0024 | 0.0017 | | | | | | 1.23 | 0.38 | 0.27 | | | 12.2 |
| 15B | 0.05 | 0.14 | 0.79 | 0.008 | 0.0040 | 5.23 | 0.039 | 0.0047 | 0.0025 | 0.003 | | | | | 0.29 | 0.45 | 0.55 | 0.03 | | 11.6 |
| 16B | 0.06 | 0.16 | 1.03 | 0.009 | 0.0081 | 5.48 | 0.031 | 0.0021 | 0.0022 | | 0.001 | | 0.0013 | | 0.48 | 0.36 | 0.31 | | | 11.1 |
| 17B | 0.11 | 0.11 | 1.33 | 0.006 | 0.0062 | 5.89 | 0.008 | 0.0066 | 0.0016 | | | | | | 0.39 | 0.41 | 0.13 | | | 14.2 |
| 19B | 0.09 | 0.08 | 1.07 | 0.008 | 0.0039 | 5.14 | 0.033 | 0.0033 | 0.0022 | | 0.002 | | | 0.0022 | | | 1.10 | | | 13.9 |
| 20B | 0.08 | 0.13 | 0.91 | 0.011 | 0.0072 | 5.19 | 0.027 | 0.0037 | 0.0018 | | | | | | 0.47 | 0.76 | 0.25 | | | 14.9 |
| 21B | 0.13 | 0.05 | 1.15 | 0.009 | 0.0042 | 5.39 | 0.038 | 0.0031 | 0.0027 | 0.002 | | | | | | 0.48 | 0.22 | | | 14.5 |
| 22B | 0.07 | 0.10 | 0.85 | 0.007 | 0.0060 | 5.01 | 0.022 | 0.0024 | 0.0019 | | 0.004 | 0.0022 | | | 0.45 | 0.66 | 0.31 | | | 12.8 |
| 24B | 0.13 | 0.11 | 1.72 | 0.014 | 0.0079 | 5.91 | 0.025 | 0.0026 | 0.0018 | | 0.002 | | | | | | | | | 6.3 |
| 25B | 0.07 | 0.12 | 1.01 | 0.010 | 0.0051 | 5.47 | 0.034 | 0.0021 | 0.0015 | | | | | | | | 0.08 | | | **3.5** |
| 26B | 0.17 | 0.05 | 1.78 | 0.013 | 0.0016 | 5.06 | 0.071 | 0.0038 | 0.0021 | | | | | | 0.16 | 0.27 | 0.21 | | | **18.1** |
| 29B | 0.06 | 0.14 | **2.55** | 0.014 | 0.0013 | 5.11 | 0.026 | 0.0031 | 0.0018 | | | | | | 0.14 | 0.07 | 0.22 | | | 11.4 |
| 101B | 0.12 | 0.15 | 1.44 | 0.009 | 0.0034 | 5.54 | 0.028 | 0.0026 | 0.0029 | | | | | | | | | | | 5.1 |
| 102B | 0.07 | 0.11 | 1.32 | 0.012 | 0.0042 | 4.89 | 0.032 | 0.0031 | 0.0032 | 0.019 | | | | | 0.25 | | 0.44 | | | 8.2 |
| 103B | 0.05 | 0.09 | 1.29 | 0.007 | 0.0028 | 5.98 | 0.033 | 0.0036 | 0.0037 | | 0.040 | | | | | 0.30 | 0.17 | 0.07 | | 8.0 |
| 104B | 0.08 | 0.16 | 1.25 | 0.008 | 0.0045 | 4.82 | 0.003 | 0.0037 | 0.0026 | 0.012 | | | | | 0.42 | | 0.50 | | | 9.6 |
| 105B | 0.11 | 0.14 | 0.96 | 0.005 | 0.0058 | 5.43 | 0.027 | 0.0042 | 0.0042 | | 0.030 | | | | | 0.35 | 0.22 | | | 10.5 |
| 106B | 0.15 | 0.13 | 1.14 | 0.007 | 0.0036 | 5.88 | 0.029 | 0.0028 | 0.0035 | | | | | | 0.35 | 0.54 | | 0.08 | | 11.9 |
| 107B | 0.07 | 0.09 | 1.64 | 0.008 | 0.0056 | 5.22 | 0.028 | 0.0046 | 0.0031 | | | | | | 0.42 | 0.42 | 0.18 | | | 13.8 |
| 108B | 0.09 | 0.14 | 1.36 | 0.006 | 0.0042 | 5.46 | 0.026 | 0.0029 | 0.0027 | 0.015 | | 0.0031 | 0.0022 | | | 0.30 | 0.34 | | | 14.5 |
| 109B | 0.06 | 0.11 | 1.28 | 0.009 | 0.0028 | 5.71 | 0.031 | 0.0038 | 0.0041 | | | | | | 0.21 | 0.34 | 0.35 | | | 12.9 |
| 110B | 0.15 | 0.14 | 1.56 | 0.005 | 0.0067 | 5.05 | 0.033 | 0.0019 | 0.0035 | | | | | | | | | | | 5.7 |
| 111B | 0.07 | 0.14 | 1.25 | 0.008 | 0.0028 | 4.91 | 0.032 | 0.0031 | 0.0025 | | | 0.0005 | | | 0.44 | | 0.53 | | | 9.4 |
| 112B | 0.12 | 0.11 | 0.92 | 0.006 | 0.0052 | 5.48 | 0.031 | 0.0038 | 0.0037 | | | | 0.0005 | | | 0.30 | 0.24 | | | 10.1 |
| 113B | 0.14 | 0.14 | 1.19 | 0.005 | 0.0030 | 5.82 | 0.025 | 0.0032 | 0.0038 | | | | | 0.0005 | 0.25 | 0.45 | | 0.08 | | 10.6 |
| 114B | 0.09 | 0.14 | 0.90 | 0.013 | 0.0032 | 5.23 | 0.032 | 0.0025 | 0.0023 | | | | | | | 0.07 | | | | **3.3** |
| 115B | 0.08 | 0.15 | 1.21 | 0.011 | 0.0029 | 5.38 | 0.031 | 0.0029 | 0.0034 | | | | | | 0.14 | | | | | **3.6** |
| 116B | 0.14 | 0.09 | 1.86 | 0.015 | 0.0023 | 5.15 | 0.035 | 0.0045 | 0.0025 | | | | | | 0.12 | 0.29 | 0.19 | | | **17.3** |
| 117B | 0.12 | 0.13 | 1.74 | 0.011 | 0.0014 | 5.23 | 0.037 | 0.0032 | 0.0033 | | | | | | 0.16 | 0.31 | 0.28 | | | **19.2** |
| 118B | 0.11 | 0.13 | 0.78 | 0.012 | 0.0082 | 5.21 | 0.037 | 0.0027 | 0.0029 | 0.002 | 0.002 | | | | | 0.45 | | | | 5.7 |
| 119B | 0.17 | 0.09 | 1.36 | 0.009 | 0.0056 | 6.08 | 0.029 | 0.0026 | 0.0041 | | 0.002 | 0.0018 | | | 0.32 | 0.38 | 0.34 | | | **25.3** |

Next, steel products were manufactured from these slabs under the manufacturing conditions listed in Table 5. "Temper heat treatment" is the heating temperature in the tempering treatment after the quenching.

**[Table 5]**

| No. | plate thickness (mm) | rolling conditions | | | Ac₃ [°C] | reheat quenching conditions | | Temper heat treatment [°C] |
|---|---|---|---|---|---|---|---|---|
| | | heating temperature [°C] | hot rolling cumulative rolling reduction ratio [%] | cooling after rolling | | reheat quenching temperature [°C] | cooling after reheating | |
| 2B | 40 | 1210 | 55 | water cooling | 699 | 1030 | water cooling | 520 |
| 4B | 19 | 1130 | 63 | water cooling | 717 | 880 | water cooling | 630 |
| 6B | 40 | 1150 | 50 | water cooling | 756 | 910 | water cooling | 620 |
| 7B | 50 | 1190 | 39 | air cooling | 760 | 930 | water cooling | 590 |
| 8B | 35 | 1180 | 60 | water cooling | 719 | **1020** | water cooling | 620 |
| 9B | 25 | 1125 | 45 | air cooling | 691 | 760 | water cooling | 580 |
| 10B | 40 | 1220 | 58 | air cooling | 774 | 880 | water cooling | - |
| 11B | 25 | 1130 | 55 | air cooling | 718 | 900 | water cooling | 530 |
| 14B | 55 | 1050 | 38 | air cooling | 753 | 890 | water cooling | 640 |
| 15B | 45 | 1170 | 42 | air cooling | 794 | 930 | water cooling | 590 |
| 16B | 60 | 1130 | 48 | water cooling | 762 | 830 | water cooling | 550 |
| 17B | 55 | 1150 | 38 | air cooling | 711 | 840 | water cooling | 520 |
| 19B | 50 | 1050 | 59 | air cooling | 793 | 880 | water cooling | 570 |
| 20B | 45 | 1130 | 50 | water cooling | 757 | 840 | water cooling | 470 |
| 21B | 40 | 1150 | 68 | air cooling | 731 | 800 | water cooling | 480 |
| 22B | 35 | 1130 | 45 | water cooling | 768 | 860 | water cooling | 600 |
| 24B | 55 | 1220 | 19 | air cooling | 700 | 850 | water cooling | 490 |
| 25B | 43 | 1150 | 43 | air cooling | 758 | 900 | water cooling | 570 |
| 26B | 50 | 1100 | 39 | water cooling | 714 | 930 | water cooling | 520 |
| 29B | 57 | 1180 | 45 | air cooling | 744 | 890 | water cooling | 590 |
| 101B | 70 | 1200 | 70 | air cooling | 723 | 850 | water cooling | - |
| 102B | 60 | 1120 | 80 | water cooling | 778 | 930 | water cooling | 590 |
| 103B | 80 | 1150 | 68 | air cooling | 755 | 900 | water cooling | 630 |
| 104B | 60 | 1200 | 75 | air cooling | 773 | 880 | water cooling | 520 |
| 105B | 50 | 1100 | 80 | water cooling | 745 | 900 | water cooling | 580 |
| 106B | 45 | 1150 | 85 | air cooling | 708 | 930 | water cooling | 610 |
| 107B | 60 | 1100 | 75 | air cooling | 744 | 870 | water cooling | 540 |
| 108B | 50 | 1250 | 80 | water cooling | 752 | 890 | water cooling | 580 |
| 109B | 45 | 1150 | 85 | air cooling | 754 | 920 | water cooling | 620 |
| 110B | 60 | 1100 | 65 | water cooling | 721 | 810 | water cooling | 520 |
| 111B | 55 | 1150 | 78 | air cooling | 779 | 860 | water cooling | 560 |
| 112B | 50 | 1200 | 83 | water cooling | 741 | 910 | water cooling | 530 |
| 113B | 45 | 1100 | 82 | air cooling | 714 | 950 | water cooling | 600 |
| 114B | 50 | 1100 | 75 | water cooling | 755 | 880 | water cooling | 540 |
| 115B | 40 | 1150 | 70 | air cooling | 748 | 900 | water cooling | 600 |
| 116B | 60 | 1200 | 70 | water cooling | 718 | 950 | water cooling | 530 |
| 117B | 50 | 1150 | 67 | air cooling | 733 | 920 | water cooling | 550 |
| 118B | 50 | 1200 | 75 | air cooling | 748 | **590** | water cooling | 480 |
| 119B | 50 | 1050 | 80 | water cooling | 691 | 830 | water cooling | 560 |

### [Measurement and Evaluation]

The microstructures and mechanical properties of the obtained steel products were measured by the above-described methods. The results are shown in Table 6. The meanings of the symbols of the microstructures are as follows. Note that the remainders of the microstructures were MA phase and ferrite.
Bu: upper bainite
BL: lower bainite
M: martensite
residual γ: residual austenite

For the toughness, the average value of the Charpy impact absorption energy at -110°C, and the average value of the Charpy impact absorption energy at -110°C after PWHT in which the holding temperature was 600°C, the holding time was 2 hours, and the rate of temperature increase and the rate of temperature decrease in the temperature region of 425°C or more were 55°C/h, respectively were measured.

**[Table 6]**

| No. | microstructure (area ratio) | | | aspect ratio average value of prior γ grains | average crystal grain diameter [µm] | YS [MPa] | TS [MPa] | YR [%] | base metal toughness KV2[J] | toughness after PWHT KV2[J] | thermal cycling toughness KV2[J] | toughness after thermal cycling and PWHT KV2 [J] | notes |
|---|---|---|---|---|---|---|---|---|---|---|---|---|---|
| | BL+M [%] | Bu+BL+M [%] | residual γ [%] | | | | | | | | | | |
| 2B | 25.2 | 92.1 | 0.0 | 1.1 | 23.2 | 569 | 654 | 87 | **146** | **122** | | | examples of present invention |
| 4B | 24.7 | 92.7 | 0.0 | 1.3 | 16.4 | 513 | 628 | 82 | 221 | 190 | | | |
| 6B | 36.2 | 92.5 | 0.1 | 1.2 | 17.3 | 572 | 661 | 87 | 248 | 222 | | | |
| 7B | 37.7 | 93.6 | 0.2 | 1.1 | 15.6 | 561 | 657 | 85 | 312 | 319 | | | |
| 8B | 34.4 | 93.2 | 0.1 | 1.0 | 22.4 | 578 | 669 | 86 | 148 | 145 | | | |
| 9B | 37.1 | 93.1 | 0.2 | 1.1 | 17.4 | 581 | 684 | 85 | 233 | 230 | | | |
| 10B | 52.7 | 95.4 | 0.4 | 1.2 | 14.1 | 621 | 734 | 85 | 281 | 278 | | | |
| 11B | 55.9 | 93.7 | 0.5 | 1.1 | 13.8 | 642 | 773 | 83 | 285 | 282 | | | |
| 14B | 67.3 | 95.2 | 0.4 | 1.4 | 14.2 | 658 | 745 | 88 | 232 | 228 | | | |
| 15B | 62.1 | 94.8 | 0.3 | 1.2 | 16.4 | 672 | 778 | 86 | 251 | 232 | | | |
| 16B | 64.3 | 95.9 | 0.4 | 1.2 | 16.7 | 651 | 739 | 88 | 233 | 218 | | | |
| 17B | 92.8 | 95.2 | 0.7 | 1.1 | 14.5 | 731 | 844 | 87 | 245 | 240 | | | |
| 19B | 91.3 | 97.1 | 0.8 | 1.3 | 15.4 | 722 | 846 | 85 | 256 | 238 | | | |
| 20B | 92.9 | 97.3 | 0.7 | 1.2 | 18.3 | 779 | 912 | 85 | 214 | 210 | | | |
| 21B | 98.2 | 98.2 | 0.6 | 1.1 | 15.6 | 736 | 857 | 86 | 252 | 232 | | | |
| 22B | 90.0 | 96.8 | 0.6 | 1.2 | 14.1 | 749 | 858 | 87 | 262 | 241 | | | |
| 24B | 38.1 | 92.3 | 0.2 | 1.4 | **27.5** | 542 | 653 | 83 | **137** | **102** | | | |
| 25B | **10.2** | **80.2** | 0.0 | 1.2 | **41.2** | 510 | **568** | 90 | **68** | **67** | | | comparative example |
| 26B | 95.3 | 98.1 | 1.3 | 1.1 | 17.0 | 891 | **992** | 90 | 159 | **119** | | | |
| 29B | 87.9 | 95.1 | 0.8 | 1.3 | 17.2 | 736 | 859 | 86 | 155 | 30 | | | |
| 101B | 26.2 | 92.3 | 0.2 | 1.1 | 19.4 | 605 | 683 | 89 | 231 | 220 | 135 | 118 | examples of present invention |
| 102B | 36.4 | 93.1 | 0.3 | 1.2 | 17.2 | 573 | 663 | 86 | 220 | 197 | 143 | 131 | |
| 103B | 34.8 | 93.0 | 0.2 | 1.1 | 17.5 | 570 | 659 | 86 | 227 | 204 | 142 | 129 | |
| 104B | 57.2 | 94.8 | 0.6 | 1.2 | 16.1 | 645 | 765 | 84 | 240 | 218 | 186 | 161 | |
| 105B | 60.2 | 95.7 | 0.7 | 1.1 | 15.6 | 674 | 770 | 88 | 252 | 228 | 192 | 175 | |
| 106B | 63.8 | 96.9 | 0.7 | 1.3 | 15.3 | 680 | 778 | 87 | 239 | 235 | 181 | 178 | |
| 107B | 93.4 | 97.1 | 1.1 | 1.2 | 14.2 | 731 | 856 | 85 | 245 | 224 | 162 | 141 | |
| 108B | 93.1 | 98.2 | 1.2 | 1.1 | 15.1 | 752 | 862 | 87 | 251 | 236 | 158 | 142 | |
| 109B | 92.0 | 98.1 | 0.9 | 1.3 | 14.8 | 744 | 858 | 87 | 254 | 250 | 172 | 169 | |
| 110B | 25.3 | 90.2 | 0.2 | 1.3 | **26.6** | 528 | 624 | 85 | **140** | **123** | 135 | 114 | |
| 111B | 55.8 | 94.3 | 0.4 | 1.2 | 13.8 | 646 | 759 | 83 | 279 | 276 | 182 | 181 | |
| 112B | 64.3 | 94.8 | 0.4 | 1.3 | 14.2 | 661 | 757 | 88 | 241 | 240 | 185 | 182 | |
| 113B | 66.1 | 95.2 | 0.5 | 1.2 | 14.3 | 674 | 775 | 86 | 255 | 251 | 195 | 192 | |
| 114B | **9.2** | **78.3** | 0.1 | 1.3 | 40.4 | 501 | **566** | 89 | 66 | 63 | 43 | 32 | comparative example |
| 115B | **10.1** | **79.1** | 0.0 | 1.2 | 39.8 | 512 | **573** | 89 | 68 | 69 | 41 | 37 | |
| 116B | 96.2 | 98.2 | 0.9 | 1.2 | 16.1 | 873 | **986** | 89 | 142 | 138 | 39 | 33 | |
| 117B | 97.3 | 98.1 | 1.2 | 1.1 | 15.8 | 884 | **995** | 89 | 138 | 135 | 36 | 32 | |
| 118B | **11.4** | **53.0** | 0.1 | 1.8 | 16.6 | 437 | **526** | 83 | 161 | 142 | 127 | 112 | |
| 119B | 96.2 | 96.8 | **1.9** | 1.2 | 18.2 | 936 | **1070** | 87 | 63 | 42 | 25 | 18 | |

Nos. 2B - 24B and 101B - 113B are Examples of the present invention, and Nos. 25B - 29B and 114B - 119B are Comparative Examples.

In No. 25B, value α was less than the lower limit value of the present disclosure, and the hardenability was insufficient, and the strength was insufficient. Sufficient low-temperature toughness also was not obtained.

In No. 26B, value α exceeded the upper limit value of the present disclosure, and the hardenability was too high, and the strength was excessive.

In No. 29B, because Mn fell outside of the upper limit, the low-temperature toughness after PWHT was low.

In Nos. 114B and 115B, value α was less than the lower limit value of the present disclosure, and the hardenability was insufficient, and the strength was insufficient. Sufficient low-temperature toughness also was not obtained.

In Nos. 116B and 117B, value α exceeded the upper limit value of the present disclosure, and the hardenability was too high, and the strength was excessive.

In No. 118B, the reheating quenching temperature was too low, and the total area ratio of the upper bainite, lower bainite and martensite was insufficient, and the strength was insufficient.

In No. 119B, value α exceeded the upper limit value of the present disclosure, and the hardenability was too high, and the strength was excessive. Further, because there was also too much residual γ, sufficient low-temperature toughness was not obtained.

In contrast to the Comparative Examples, in the Examples of the present invention, the chemical compositions and microstructures of the steel products were controlled appropriately, and the tensile strengths were in the appropriate range of 615 MPa or more and 930 MPa or less. In addition, low-temperature toughness at -110°C of 100 J or more was obtained regardless of whether before or after PWHT. In particularly suitable structures of the present disclosure, low-temperature toughness at -110°C of 150 J or more was obtained regardless of whether before or after PWHT.

### Industrial Applicability

The steel products relating to the present disclosure can be used mainly for transport tanks of liquefied carbon dioxide. Further, the steel products relating to the present disclosure can also be used in other welded structures such as buildings, bridges, ships, pipelines, offshore structures, pressure vessels and tanks.

The disclosures of Japanese Patent Application No. 2023-042399 and Japanese Patent Application No. 2023-042402 filed on March 16, 2023 are, in their entireties, incorporated by reference into the present specification. All publications, patent applications, and technical standards mentioned in the present specification are incorporated by reference into the present specification to the same extent as if such individual publication, patent application, or technical standard was specifically and individually put forth herein.

## Claims

1. A steel product having a chemical composition comprising, in mass%,
C: 0.03% or more and 0.20% or less,
Si: 0.01% or more and 0.50% or less,
Mn: 0.10% or more and 2.00% or less,
P: 0.025% or less,
S: 0.0250% or less,
Ni: 4.51% or more and 6.10% or less,
Al: 0.001% or more and 0.100% or less,
O: 0.0100% or less,
N: 0.0100% or less,
Cu: 0 - 1.50%,
Cr: 0 - 3.00%,
Mo: 0 - 2.00%,
B: 0 - 0.0050%,
Nb: 0 - 0.050%,
Ti: 0 - 0.050%,
V: 0 - 0.10%,
Mg: 0 - 0.0200%,
Ca: 0 - 0.0200%,
REM: 0 - 0.0200%,
balance: Fe and impurities,
and in which α expressed by following formula (1) is 5.0 or more and 16.0 or less,
wherein:
a tensile strength is 615 MPa or more and 930 MPa or less, and
a microstructure of a region that is 1/4 of a thickness in a thickness direction from a surface of the steel product contains lower bainite and martensite, and a total of area ratios of the lower bainite and the martensite is 15.0% or more, and a total of area ratios of upper bainite and the lower bainite and the martensite is 90.0% or more, and an area ratio of residual austenite is less than 1.7%. α = 0.50 × √[C] × (1+0.64[Si]) × (1+4.10[Mn]) × (1+0.27[Cu]) × (1+0.52[Ni]) × (1+2.33[Cr]) × (1+3.14[Mo])
wherein [element symbol] in formula (1) represents content (mass%) of a respectively corresponding element contained in the steel product, and, in a case in which an element is not contained, zero is substituted in therefor.

2. The steel product of Claim 1, wherein, in the microstructure of the region that is 1/4 of the thickness in the thickness direction from the surface of the steel product, an average crystal grain diameter is 20.0 µm or less.

3. The steel product of Claim 1 or Claim 2, wherein a Charpy impact absorption energy at -110°C is 150 J or more.

4. The steel product of any one of Claim 1 through Claim 3, wherein, in a case in which a heat treatment, in which a rate of temperature increase and a rate of temperature decrease in a temperature region of 425°C or more are 55°C/h and temperature is held for 2 hours at 600°C, is carried out on the steel product, a Charpy impact absorption energy at -110°C of portions where the heat treatment has been carried out is 150 J or more.

5. The steel product of any one of Claim 1 through Claim 4, wherein an aspect ratio of prior austenite crystal grains of the region that is 1/4 of the thickness in the thickness direction from the surface of the steel product is 1.5 or more.

6. The steel product of any one of Claim 1 through Claim 4, wherein an aspect ratio of prior austenite crystal grains of the region that is 1/4 of the thickness in the thickness direction from the surface of the steel product is less than 1.5.
